



US005145759A

# United States Patent [19]

Terrell et al.

[11] Patent Number: 5,145,759

[45] Date of Patent: Sep. 8, 1992

[54] ELECTROPHOTOGRAPHIC RECORDING MATERIAL

[75] Inventors: David R. Terrell, Lint; Stefaan K. De Meutter, Zandhoven; Marcel J. Monbaliu, Mortsel, all of Belgium

[73] Assignee: AGFA-Gevaert, N.V., Mortsel, Belgium

[21] Appl. No.: 509,248

[22] Filed: Apr. 16, 1990

[30] Foreign Application Priority Data

Apr. 21, 1989 [BE] Belgium ..... 89201035.6

[51] Int. Cl.<sup>5</sup> ..... G03G 5/047; G03G 5/09

[52] U.S. Cl. ..... 430/58; 430/59;  
430/83; 430/95; 430/900; 430/74; 430/78;  
430/79

[58] Field of Search ..... 430/74, 78, 79, 83,  
430/95, 900, 58, 59

[56] References Cited

U.S. PATENT DOCUMENTS

3,798,031 3/1974 Janssens et al. ..... 430/78 X  
3,912,509 10/1975 Janssens et al. ..... 430/79  
4,264,695 4/1981 Kozima et al. ..... 430/83 X  
4,755,443 7/1988 Suzuki et al. ..... 430/78 X

4,882,253 11/1989 Kato et al. ..... 430/59  
4,923,774 5/1990 Van der Auweraer et al. .... 430/59

Primary Examiner—Roland Martin  
Attorney, Agent, or Firm—Breiner & Breiner

[57] ABSTRACT

An electrophotographic recording material comprising on an electrically conductive support a negatively chargeable photoconductive recording layer which contains in an electrically insulating organic polymer binder material at least one photoconductive n-type pigment substance and at least one p-type photoconductive charge transport substance as defined herein by a general formula (I) to (V), wherein said layer has a thickness in the range of 4 to 40  $\mu$ m and comprises 8 to 80% by weight of said n-type pigment substance and 0.01 to 40% by weight of said p-type charge transport substance that is molecularly distributed in said electrically insulating organic polymeric binder material that has a volum resistivity of at least  $10^{14}$  Ohm-m, and wherein said recording layer in electrostatically charged state requires for 10% and 90% discharge respectively exposures to conductivity increasing electromagnetic radiation that differ by a factor 4.5 or less.

17 Claims, 21 Drawing Sheets

FIG. 1

























Fig. 12



















## ELECTROPHOTOGRAPHIC RECORDING MATERIAL

### DESCRIPTION

The present invention relates to a photosensitive recording material suitable for use in electrophotography.

In electrophotography photoconductive materials are used to form a latent electrostatic charge image that is developable with finely divided colouring material, 10 called toner.

The developed image can then be permanently affixed to the photoconductive recording material, e.g. photoconductive zinc oxide-binder layer, or transferred from the photoconductor layer, e.g. selenium layer, onto a receptor material, e.g. plain paper and fixed thereon. In electrophotographic copying and printing systems with toner transfer to a receptor material the photoconductive recording material is reusable. In order to permit a rapid multiple printing or copying a photoconductor layer has to be used that rapidly losses its charge on photo-exposure and also rapidly regains its insulating state after the exposure to receive again a sufficiently high electrostatic charge for a next image formation. The failure of a material to return completely to its relatively insulating state prior to succeeding charging/imaging steps is commonly known in the art as "fatigue".

The fatigue phenomenon has been used as a guide in the selection of commercially useful photoconductive materials, since the fatigue of the photoconductive layer limits the copying rates achievable.

Another important property which determines whether a particular photosensitive recording material is suitable for electrophotographic systems is its discharge-exposure relationship. Conventional recording materials on the basis of an electrostatically charged photoconductive layer exhibit a fairly gradual increase in discharge as a function of increasing exposure to photoconductivity increasing electromagnetic radiation. The radiation dose, also called exposure, required for 10% and 90% discharge differs normally by factors of about 10 to 40 depending on the choice of photoconductive recording material.

Electrophotographic copying systems wherein such photoconductive recording materials are used in the reproduction of halftone image originals, i.e. images composed of equi-dense screen dots in which density variation is obtained only by varying dot frequency or by varying dot size and dot frequency, yield images of degraded quality (resolution) when compared with images obtained on lith-type silver halide emulsion materials.

Electrophotographic printing systems operating with scanning light sources such as analog-signal or digital-signal modulated laser beams or light emitting diodes with such photoconductive recording materials likewise produce degraded prints due to the enhancement of background and the blurring of the dots as a result of each dot having a halo caused by the unsharp edge of 60 the writing beam.

It is therefore desirable for high quality electrophotographic copying and printing to have a photoconductive recording material with a sharp decrease in charge expressed in voltage (V) (as a result of sharp increase in conductivity) within a narrow range of photo-exposure dose (E) [ $E = \text{photon-intensity (I)} \times \text{time (t)}$ ]. More explicitly it is desirable in order to avoid said image quality

degradation to work with a photoconductive recording material with which the exposures required for 10% and 90% discharge differ by a factor of only 4.5 or less.

Another important property which determines whether or not a particular photoconductive material is suited for electrophotographic copying is its photosensitivity that must be high enough for use in copying apparatus operating with fairly low intensity light reflected from the original.

Commercial usefulness further requires that the photoconductive layer has a chromatic sensitivity that matches the wavelength(s) of the light of the light source, e.g. a laser or has panchromatic sensitivity when white light is used e.g. to allow the reproduction of all colours in balance.

Intensive efforts have been made to satisfy said requirements, e.g. the spectral sensitivity of selenium has been extended to the longer wavelengths of the visible spectrum by making alloys of selenium, tellurium and arsenic. In fact selenium-based photoconductors remained for a long time the only really useful photoconductors although many organic photoconductors were discovered.

The first generation of organic photoconductors consisted of single layers in which a polymeric charge transport material such as poly(N-vinylcarbazole) (PVK) or charge transport molecules such as the 1,2-dihydro-2,2,4-trimethylquinoline derivatives described in U.S. Pat. Nos. 3,830,647 and 3,832,171 dissolved in an inert polymeric binder such as a polycarbonate were sensitized with dissolved dyes or dispersed pigment particles. Examples of the latter are the so-called "photoemission active material" (PEAM) layers such as those disclosed by Regensburger and Jakubowski in U.S. Pat. No. 3,877,935 for novel xerographic plates containing photoinjecting polynuclear quinone pigments including 4,10-dibromoanthrone in concentrations of 0.1 to 5 percent by volume with 5 to 99 percent by volume of photoconductor material. Hackett also described such layers in 1971 in the Journal of Chemical Physics, Volume 55, page 3178 consisting of 25 wt % X-phthalocyanine dispersed in poly(N-vinylcarbazole).

With 5 to 10  $\mu\text{m}$  thick PEAM-layers consisting of about 40% by weight of the p-type charge transport material 2,4-bis(4-N,N-diethylaminophenyl)oxadiazole, 0.5 to 10% by weight of N,N'-dimethylperylimide in a binder [ref. Chemiker Zeitung 106, 313 (1982)] Wiedemann observed photosensitivities expressed as half-value voltage drop exposures ( $I_{0.5} \cdot t_1$ ) of 50 to 100  $\text{mJ/m}^2$  for positive and negative charging.

Nakazawa, Muto and Tsutsumi in 1988 [Japan Hard-copy Proceedings May 16-18, 1988] described a positively chargeable 18  $\mu\text{m}$  PEAM-layer with metal-free phthalocyanine and N,N'-bis(3,5-xylyl)perylimide as the sensitizing pigments and a charge carrier transport material, which exhibited optimal photosensitivity ( $I_{0.5} \cdot t_1$ ) of 238  $\text{mJ/m}^2$  at a metal-free phthalocyanine concentration of 0.3% by weight, a N,N'-bis(3,5-xylyl)perylimide concentration of 5.4% by weight and a charge carrier transport material concentration of 40.4% by weight.

Such monolayer organic photoconductors were less interesting than selenium-photoconductors, because of their poorer sensitivity, their very flat response to increasing exposure dose and their rather large fatigue.

However, the discovery that 2,4,7-trinitro-9-fluorenone (TNF) in poly(N-vinylcarbazole) (PVCz) formed a charge-transfer complex strongly improving the photosensitivity (ref. U.S. Pat. No. 3,484,237) opened the way for the use of organic photoconductors in copying machines that could compete with the selenium-based machines.

TNF acts as an electron acceptor whereas PVCz serves as electron donor. Films consisting of said charge transfer complex with TNF:PVCz in 1:1 molar ratio are dark brown, nearly black and exhibit high charge acceptance and low dark decay rates. However, the exposures required for 10% and 90% discharges differed by more than a factor of 10. Overall photosensitivity is comparable to that of amorphous selenium (ref. Schaffert, R. M. IBM J. Res. Develop., 15, 75 (1971)).

Subsequently single layer photoconductive materials containing aggregates of photoconductors which are both positively and negatively chargeable were developed, e.g. consisting of ternary systems comprising a thio-pyrilium dye, a polycarbonate polymer and an aromatic molecule such as bis(4-N,N-diethylamino-2-methyl-phenyl)-phenylmethane. In 1979 Mey et al [J.Appl.Phys. 50, 8090 (1979)] published surface potential-exposure characteristics for such photoconductive recording materials with both negative and positive charging and for both emission-limited discharge and high-intensity flash. In all cases the exposures required for 10% and 90% discharges differed by more than a factor of 10.

A further search led to the discovery that if the sensitizing pigment in PEAM-layers were cast in a thin layer adjacent to a thicker layer solely consisting of transport molecules dissolved in an inert polymer binder or a polymeric charge transport material sensitivity comparable with selenium-photoconductors together with a much steeper response to increase in exposure dose and a much reduced fatigue were observed. Hackett showed this in 1971 [J.Chem.Phys. 55, 3178 (1971)] for the system X-phthalocyanine and PVK. Hackett found that photoconductivity was due to field dependent photogeneration of electron-hole pairs in the phthalocyanine and hole injection into the PVCz. The transport of the positive charges, i.e. positive hole-conduction proceeded easily in the PVCz layer. From that time on much research has been devoted to developing improved photoconductive systems wherein charge generation and charge transport materials are separate in two contiguous layers (see e.g. U.K. Pat No. 1,577,859). However, such functionally separated double layer photoconductors although generally exhibiting a steeper response to increasing exposure doses than single layer photoconductors still exhibit exposure doses for 10 and 90% discharge differing by a factor of 10 or more as shown in comparative examples furtheron.

It is an object of the present invention to provide electrophotographic recording materials with high photosensitivity which after being charged obtain a very sharp decrease in voltage  $[\Delta V]$  within a particular narrow range  $[\Delta E]$  of photo-exposure doses, viz. wherein the photo-exposure doses required for 10% and 90% discharge differ by a factor of 4.5 or less.

Other objects and advantages of the present invention will appear from the further description and examples.

In accordance with the present invention an electrophotographic recording material is provided which comprises on an electrically conductive support a negatively chargeable photoconductive recording layer

which contains in an electrically insulating organic polymeric binder material at least one photoconductive n-type pigment substance and one or more p-type photoconductive charge transport substances, wherein said layer has a thickness in the range of 4 to 40  $\mu\text{m}$  and comprises 8 to 80% by weight of said n-type pigment substance and 0.01 to 40% by weight of said p-type charge transport substance that is molecularly distributed in said electrically insulating organic polymeric binder material that has a volume resistivity of at least  $10^{14}$  Ohm-m, and wherein said recording layer in electrostatically charged state requires for 10% and 90% discharge respectively exposures to conductivity increasing electromagnetic radiation that differ by a factor 4.5 or less, and wherein at least one p-type charge transport substance corresponds to a following general formula (I) to (V):



wherein:

R represents hydrogen or an aliphatic or cycloaliphatic group, e.g. a saturated aliphatic group or an unsaturated aliphatic group, including these groups substituted by non-ionic substituents,

each of R<sup>1</sup> and R<sup>2</sup> (same or different) represents a C<sub>1</sub>-C<sub>6</sub> alkyl group, e.g. methyl, ethyl, n-propyl, iso-propyl, n-butyl, isobutyl, n-pentyl and n-hexyl, or an aryl group, e.g. phenyl, and

Z represents the atoms necessary to close an adjacent aromatic nucleus, e.g. benzene nucleus, or aromatic ring system including such nucleus or ring system substituted with one or more substituents of non-ionic character, e.g. substituted with one or more alkyl groups, one or more halogen atoms, e.g. F, Cl, Br or I, one or more cyano groups, nitro groups, alkoxy groups, e.g. methoxy, or amino groups, e.g. a monoalkylamino or a dialkylamino group, (a) hydrazone group(s), e.g. (a) formyl-1,1-diphenyl hydrazone group, a formyl-1-methyl-1-phenyl hydrazone group, (an) azo group(s), e.g. an azobenzene group, (an) enamine group(s), e.g. a group obtained by condensation of formaldehyde with a primary amine group;



wherein:

X is a bivalent aliphatic or cycloaliphatic group, e.g. of the type that can be introduced by alkylation, e.g. an alkylene group, preferably an ethylene group, a substituted alkylene group or an alkylene chain interrupted by a bivalent aromatic group, e.g. a phenylene, naphthalene or anthracene group, or a bivalent aliphatic group wherein at least two car-

bon atoms are linked through a hetero-atom selected from the group consisting of oxygen, sulphur or nitrogen wherein nitrogen is substituted with a monovalent hydrocarbon group, e.g. an aryl group, and

R<sup>1</sup>, R<sup>2</sup> and Z have the same significance as described for general formula (I);



(III)

5

10

15

wherein:

R<sup>11</sup> is —NR<sup>4</sup>R<sup>5</sup>, wherein each of R<sup>4</sup> and R<sup>5</sup> (same or different) represents hydrogen, an aliphatic or cycloaliphatic group including said groups in substituted form, e.g. methyl or benzyl, or an aryl group e.g. phenyl, or

R<sup>4</sup> and R<sup>5</sup> together represent the atoms necessary to complete a nitrogen-containing ring including such ring in substituted form, e.g. a carbazolyl ring, or

R<sup>11</sup> is —N=N—Cp, wherein Cp is an azocoupler residue such as from an aromatic amine or an aromatic hydroxy compound used in azo coupling, or

R<sup>11</sup> is —N=CH—R<sup>6</sup>, wherein R<sup>6</sup> represents an aliphatic or cycloaliphatic group including said groups in substituted form, e.g. methyl or benzyl, or an aryl group, e.g. phenyl,

Ar presents a bivalent aromatic group including said group in substituted form, e.g. a phenylene group or a biphenylene group, and

each of R<sup>12</sup> and R<sup>13</sup> (same or different) represents hydrogen, halogen, an alkyl group, an alkoxy group or a —NR<sup>7</sup>R<sup>8</sup> group, wherein each of R<sup>7</sup> and R<sup>8</sup> (same or different) represents an aryl group, a C<sub>1</sub>—C<sub>10</sub> alkyl group including such alkyl group in substituted form, e.g. an aralkyl group, preferably methyl, ethyl or benzyl;

6  
R<sup>12</sup>, R<sup>13</sup> and R<sup>14</sup> have the same significance as described for general formula (III);



wherein:

R<sup>21</sup> represents a —NR<sup>23</sup>R<sup>24</sup> group, wherein each of R<sup>23</sup> and R<sup>24</sup> (same or different) represents a C<sub>1</sub>—C<sub>10</sub> alkyl group including said alkyl group in substituted form, e.g. an aralkyl group, preferably a benzyl group, or an alkoxy carbonyl substituted C<sub>1</sub>—C<sub>10</sub> alkyl group, a cycloalkyl group, or an aryl group, and

R<sup>22</sup> represents hydrogen, an alkyl group including a substituted alkyl group, e.g. methyl, alkoxy carbonyl substituted alkyl or halogen, e.g. chlorine.

According to an embodiment of a recording material of the present invention the recording layer contains a mixture of different p-type charge transport substances including at least one substance according to a general formula (I) to (V) defined hereinbefore. In said recording material the mixed charge transport substances have half-wave oxidation potentials, that do not differ by more than 0.4 V.

The half-wave oxidation potential measurements are carried out using a polarograph with rotating (500 rpm) platinum disc electrode and standard saturated calomel electrode (s.c.e.) at room temperature (20° C. using a product concentration of 10<sup>-4</sup> mole and an electrolyte (tetrabutylammonium perchlorate) concentration of 0.1 mole in spectroscopic grade acetonitrile. Ferrocene was used as a reference substance having a half-wave oxida-



(IV)

wherein:

X is a bivalent aliphatic or cycloaliphatic group of the type that can be introduced by alkylation e.g. an alkylene group, preferably an ethylene group, a substituted alkylene group or an alkylene group interrupted by a bivalent aromatic group, e.g. a phenylene, naphthalene or anthracene group, or a bivalent aliphatic group wherein at least two carbon atoms are linked through a hetero atom selected from the group consisting of oxygen, sulphur or nitrogen wherein nitrogen is substituted with a monovalent hydrocarbon group, e.g. an aryl group, and

tion potential of +0.430 V.

Examples of and preparation of p-type charge transport substances according to the above general formulae (I) or (II) are described in published European Patent Application 0 347 960.

Examples of and preparation of p-type charge transport substances according to the above general formulae (III) or (IV) are described in published European Patent Application 0 347 967.

Examples of and preparation of p-type charge transport substances according to the above general formula

(V) are described in published European Patent Application 0 349 034.

Examples of suitable p-type charge transport substances that can be used dissolved in a binder, e.g. polycarbonate resin, in admixture with one or more p-type charge transport substances according to a general formula (I) to (V) as described above are low molecular weight substances from one of the following classes:

- i) triphenylamines, e.g. tris(p-tolyl)amine as disclosed e.g. in U.S. Pat. No. 3,180,730;
- ii) tetra-N,N,N',N'-tetraphenylbenzidines, e.g. N,N'-diphenyl-N,N'-bis (3-methyl-phenyl)benzidine as disclosed e.g. in U.S. Pat. No. 4,265,990;
- iii) hydrazones, e.g. 4-N,N'-diethylaminobenzaldehyde-1',1'-diphenyl hydrazone as disclosed e.g. in U.S. Pat. No. 4,150,987, 3-formyl-N-ethyl carbazole-1'-phenyl-1'-methyl hydrazone as disclosed e.g. in DE-OS 2 939 483 and 3-formyl-N-ethylcarbazole-1',1'-diphenyl hydrazone as disclosed e.g. in DE-OS 3 020 108;
- iv) pyrazolines, e.g. as disclosed in U.S. Pat. No. 3,837,851;
- v) oxadiazoles, e.g. 2,5-bis(4-N,N-diethylaminophenyl) oxadiazole-1,3,4 as disclosed e.g. in DBP 2 237 539;
- vi) triarylmethanes, e.g. bis(4-N,N-diethylamino-2-methyl)phenyl methane as disclosed e.g. in DBP 1 237 900 and U.S. Pat. No. 4,127,412; or polymeric p-type charge transport substances from e.g. one of the following classes:
  - i) poly(N-vinylcarbazoles)
  - ii) poly(vinylpolycyclic aromatics), e.g. poly(9-vinylanthracene);
  - iii) pyrene-formaldehyde condensation polymers, e.g. as disclosed in DBP 1 218 286;
  - iv) polyxylylenes e.g. as disclosed in J. Signal AM 5, 2, 111 (1977);
  - v) polymeric 1,2-dihydro-2,2,4-trimethylquinoxalines;
  - vi) polymeric tetraphenylbenzidines and tri-phenylamines, e.g. as disclosed in EP 295 113, 295 115, 295 125, 295 126 and 295 127.

The n-type pigment may be inorganic or organic and may have any colour including white. It is a finely divided substance dispersible in the organic polymeric binder of said photoconductive recording layer.

Optionally the support of said photoconductive recording layer is pre-coated with an adhesive and/or a blocking layer (rectifier layer) reducing or preventing positive hole charge injection from the conductive support into the photoconductive recording layer, and optionally the photoconductive recording layer is over-coated with an outermost protective layer, more details about said layers being given furtheron.

In accordance with a preferred embodiment said photoconductive recording layer has a thickness in the range of 5 to 35  $\mu\text{m}$  and contains 10 to 70% by weight of said n-type pigment material(s) and 1 to 30% by weight of said p-type charge transport material(s).

In accordance with more preferred embodiments said recording layer has a thickness in the range of 5 to 35  $\mu\text{m}$  and contains 50 to 80% by weight of said n-type pigment substance and 0.01 to 10% by weight of said p-type charge transport substance(s), or said recording layer has a thickness in the range of 5 to 35  $\mu\text{m}$  and contains 15 to 30% by weight of said n-type pigment substance and between 20 and 30% by weight of said p-type charge transport substance(s).

By the term "n-type" material is understood a material having n-type conductance, which means that the photocurrent ( $I_n$ ) generated in said material when in contact with an illuminated transparent electrode having negative electric polarity is larger than the photocurrent ( $I_p$ ) generated when in contact with a positive illuminated electrode ( $I_n/I_p > 1$ ).

By the term "p-type" material is understood a material having p-type conductance, which means that the photocurrent ( $I_p$ ) generated in said material when in contact with an illuminated transparent electrode having positive polarity is larger than the photocurrent ( $I_n$ ) generated when in contact with a negative illuminated electrode ( $I_p/I_n > 1$ ), [ref. Hans Meier—Organic Semiconductors -Dark- and Photoconductivity of Organic Solids—Verlag Chemie (1974), p. 410, point 3.]

The electrically insulating binder has preferably a volume resistivity which is not higher than  $10^{16}$  Ohm-m.

Examples of n-type pigments dispersible in the binder of the negatively chargeable recording layer of the electrophotographic recording material according to the present invention are organic pigments from one of the following classes:

- a) perylimides, e.g. C.I. 71 130 (C.I.=Colour Index) described in DBP 2 237 539,
- b) polynuclear quinones, e.g. anthranthrones such as C.I. 59 300 described in DBP 2 237 678,
- c) quinacridones, e.g. C.I. 46 500 described in DBP 2 237 679,
- d) naphthalene 1,4,5,8-tetracarboxylic acid derived pigments including the perinones, e.g. Orange GR, C.I. 71 105 described in DBP 2 239 923,
- e) n-type indigo and thioindigo dyes, e.g. Pigment Red 88, C.I. 73 312 described in DBP 2 237 680,
- f) perylene 3,4,9,10-tetracarboxylic acid derived pigments including condensation products with o-diamines as described e.g. in DAS 2 314 051,
- g) n-type polyazo-pigments including bisazo-, trisazo- and tetrakisazo-pigments, e.g. N,N'-bis(4-azobenzyl)perylimide.

For use as binder material resins are selected preferably on the basis of optimal mechanical strength, adherence to any adjacent layer(s) and favourable electrical properties and if the active layer is at the same time the outermost layer also on the basis of reducing their surface energy and frictional coefficient in order to improve the resistance of the surface of the photosensitive recording material to toner smearing and abrasion and the ease with which untransferred toner can be removed.

Suitable binder material for use in the recording material of the present invention are organic resin materials, e.g. cellulose esters, acrylate and methacrylate resins, e.g. cyanoacrylate resin, polyvinyl chloride, copolymers of vinyl chloride, e.g. copolyvinyl chloride-acetate and copolyvinylchloride/maleic anhydride, polyester resins, e.g. copolymers of isophthalic acid and terephthalic acid with glycol, aromatic polycarbonate resins and polyester carbonate resins.

The recording layer as outermost layer can be endowed with a low surface adhesion and a low frictional coefficient by the incorporation therein of a resin comprising a block copolyester or copolycarbonate having a fluorinated polyether block as described in U.S. Pat. No. 4,772,526.

A polyester resin particularly suited for use in combination with aromatic polycarbonate binders is DYNAPOL L 206 (registered trade mark of Hüls A.G. W-Ger-

many for a copolyester of terephthalic acid and isophthalic acid with ethylene glycol and neopentyl glycol, the molar ratio of tere- to isophthalic acid being 3/2). Said polyester resin improves the adherence to aluminium that may form a conductive coating on the support of the recording material.

Suitable aromatic polycarbonates can be prepared by methods such as those described by D. Freitag, U. Grigo, P. R. Müller and W. Nouverté in the Encyclopedia of Polymer Science and Engineering, 2nd ed., Vol. II, pages 648-718, (1988) published by Wiley and Sons Inc., and have one or more repeating units within the scope of the following general formula:



wherein:

X represents S, SO<sub>2</sub>,



R<sup>31</sup>, R<sup>32</sup>, R<sup>33</sup>, R<sup>34</sup>, R<sup>37</sup>, and R<sup>38</sup> each represents (same or different) hydrogen, halogen, an alkyl group or an aryl group, and

R<sup>35</sup> and R<sup>36</sup> each represent (same or different) hydrogen, an alkyl group, an aryl group or together represent the necessary atoms to close a cycloaliphatic ring, e.g. cyclohexane ring.

Aromatic polycarbonates having a molecular weight in the range of 10,000 to 200,000 are preferred. Suitable polycarbonates having such a high molecular weight are sold under the registered trade mark MAKROLON of Farbenfabriken Bayer AG, W-Germany.

MAKROLON CD 2000 (registered trade mark) is a bisphenol A polycarbonate with molecular weight in the range of 12,000 to 25,000 wherein R<sup>31</sup>=R<sup>32</sup>=R<sup>33</sup>=R<sup>34</sup>=H; X is R<sup>35</sup>-C-R<sup>36</sup> with R<sup>35</sup>=R<sup>36</sup>=CH<sub>3</sub>.

MAKROLON 5700 (registered trade mark) is a bisphenol A polycarbonate with molecular weight in the range of 50,000 to 120,000 wherein R<sup>31</sup>=R<sup>32</sup>=R<sup>33</sup>=R<sup>34</sup>=H, X is



with R<sup>35</sup>=R<sup>36</sup>=CH<sub>3</sub>.

Further useful binder resins are silicone resins, polystyrene and copolymers of styrene and maleic anhydride and copolymers of butadiene and styrene.

The photoconductive recording layer may contain further additives such as spectral sensitizing agents known in the art, e.g. (poly)methine dyes, for enlarging the spectral sensitivity of the applied photoconductive compounds, and compounds acting as stabilising agents

against deterioration by ultra-violet radiation, so-called UV-stabilizers, e.g. benzotriazoles.

For controlling the viscosity of the coating compositions and controlling their optical clarity silicone oils may be used.

An adhesive layer and/or blocking layer being optionally present between the conductive support and the photoconductive recording layer may contain or consist of one or more of e.g. a polyester, a polyamide, nitrocellulose, hydrolysed silane, or aluminium oxide. The total layer thickness of said layer(s) is preferably not more than 2 micron.

The photoconductive recording layer may be coated optionally with a thin outermost protective layer to endow its surface with improved abrasion resistance, a reduced frictional coefficient, reduced tendency to toner smearing and more easy removal of untransferred toner. Preferably said outermost layer is a binder layer containing at least one p-type transport substance being not admixed with said n-type photoconductive pigment(s). The thickness of said outermost layer is preferably not larger than 7 µm, more preferably 2 µm. The concentration of said p-type charge transport substance(s) in the outermost layer preferably does not exceed 50 wt % to avoid excessive abrasion in use.

Suitable resins for use in a protective layer with low friction coefficient are block copolyester or copolycarbonate resins having a fluorinated polyether block as described e.g. in U.S. Pat. No. 4,772,526, or are copolymers of tetrafluoroethylene or hexafluoropropene, optionally in combination with resins compatible therewith, e.g. cellulose esters, acrylate and methacrylate resins, e.g. cyanoacrylate resin, polyvinyl chloride, copolymers of vinyl chloride, e.g. copolyvinyl chloride/acetate and copolyvinyl chloride/maleic anhydride, polyester resins, aromatic polycarbonate resins or polyester-carbonate resins.

The conductive support may be made of any suitable conductive material. Typical conductors include aluminum, steel, brass and paper and resin materials incorporating or coated with conductivity enhancing substances, e.g. vacuum-deposited metal, dispersed carbon black, graphite and conductive monomeric salts or a conductive polymer, e.g. a polymer containing quaternized nitrogen atoms as in Calgon Conductive polymer 261 (trade mark of Calgon Corporation, Inc., Pittsburgh, Pa., U.S.A.) described in U.S. Pat. No. 3,832,171.

The support may be in the form of a foil, web or be part of a drum.

An electrophotographic recording process according to the present invention comprises the steps of:

- (1) overall negatively electrostatically charging, e.g. with corona-device, the recording material of the present invention,
- (2) image-wise photo-exposing the recording material according to the present invention thereby obtaining a latent electrostatic image.

The development of the latent electrostatic image commonly occurs preferably with finely divided electrostatically attractable material, called toner particles that are attracted by coulomb force to the electrostatic charge pattern. The toner development is a dry or liquid toner development known to those skilled in the art.

In positive-positive development toner particles deposit on those areas of the charge carrying surface which are in positive-positive relation to the original image. In reversal development, toner particles migrate

and deposit on the recording surface areas which are in negative-positive image value relation to the original. In the latter case the areas discharged by photo-exposure obtain by induction through a properly biased developing electrode a charge of opposite charge sign with respect to the charge sign of the toner particles so that the toner becomes deposited in the photo-exposed areas that were discharged in the imagewise exposure (ref.: R. M. Schaffert "Electrophotography"—The Focal Press—London, New York, enlarged and revised edition 1975, p. 50-51 and T. P. Maclean "Electronic Imaging" Academic Press—London, 1979, p. 231).

According to a particular embodiment electrostatic charging, e.g. by corona, and the imagewise photo-exposure proceed simultaneously.

Residual charge after toner development may be dissipated before starting a next copying cycle by overall exposure and/or alternating current corona treatment.

Recording materials according to the present invention depending on the spectral sensitivity of the photoconductive recording layer may be used in combination with all kinds of photon-radiation, e.g. light of the visible spectrum, infra-red light, near ultra-violet light and likewise X-rays when electron-positive hole pairs can be formed by said radiation in the recording layer. Thus, they can be used in combination with incandescent lamps, fluorescent lamps, laser light sources or light emitting diodes by proper choice of the spectral sensitivity of the charge generating substance or mixtures thereof.

The toner image obtained may be fixed onto the recording material or may be transferred to a receptor material to form thereon after fixing the final visible image.

A recording material according to the present invention showing a particularly low fatigue effect can be used in recording apparatus operating with rapidly following copying cycles including the sequential steps of overall charging, imagewise exposing, toner development and toner transfer to a receptor element.

The evaluations of electrophotographic properties determined on the recording materials of the following examples relate to the performance of the recording materials in an electrophotographic process with a reusable photoreceptor. The measurements of the performance characteristics were carried out as follows:

Two procedures were used for evaluating the discharge as a function of exposure: a routine sensitometric measurement in which the discharge was obtained for 8 different exposures including zero exposure and a more refined measurement in which the discharge was obtained for 360 different exposures in a single drum rotation.

In the routine sensitometric measurement the photoconductive recording sheet material was mounted with its conductive backing on an aluminium drum which was earthed and to which the conductive backing had been connected. The drum was rotated at a circumferential speed of 5 cm/s and the recording material sequentially charged with a negative corona at a voltage of -4.6 kV operating with a corona current of about 1  $\mu$ A per cm of corona wire, exposed (simulating imagewise exposure) with monochromatic light obtained from a monochromator positioned at the circumference of the drum at an angle of 45° with respect to the corona source for 400 ms, the voltage measured with an electrometer probe positioned at an angle of 180° with re-

spect to the corona source and finally post-exposed with a halogen lamp producing 54,000 mJ/m<sup>2</sup> positioned at an angle of 270° with respect to the corona source before starting a new copying cycle.

Each measurement consisted of 40 copying cycles with the exposure being changed every 5 copying cycles by using a constant light intensity ( $I_0$ ) initially using no light attenuating filter, and thereupon sequentially a filter with an optical density of 0.5, a filter with an optical density of 1.0, filters with a total optical density of 1.5, a filter with an optical density of 2.0, filters with a total optical density of 2.5, filters with a total optical density of 3.0 and finally a shutter to shut off the exposing light. This gives the discharges for 8 predetermined exposures. The charging level (CL) was taken as the average charging level over the last 5 cycles at zero exposure.

In the refined sensitometric measurement the photoconductive recording sheet material is mounted on an aluminium drum as described above. The drum was rotated at a circumferential speed of 2 cm/s and the recording material sequentially charged with a negative corona at a voltage of -4.3 kV operating with a corona current of ca 0.5  $\mu$ A per cm of corona wire, exposed (simulating image-wise exposure) with monochromatic light obtained from a monochromator positioned at the circumference of the drum at an angle of 40° with respect to the corona source for 500 ms, the voltage measured with an electrometer probe positioned at an angle of 90° with respect to the corona source and finally post-exposed with a halogen lamp producing 2,000 mJ/m<sup>2</sup> positioned at an angle of 300° with respect to the corona source before starting a new copying cycle. Each measurement consisted of a single copying cycle in which a density disc with continuously varying optical density from an optical density of 0 to an optical density of 2.1 over a sector of 210° was rotated in front of the monochromator synchronously with the rotation of the drum with the surface potential being measured every degree of rotation. This gives the discharges for 360 predetermined exposures and hence a complete sensitometric curve, whereas the routine measurement only gives 8 points on that curve.

For a given corona voltage, corona current, separating distance of the corona wires to recording surface and drum circumferential speed the charging level CL is only dependent upon the thickness of the charge transport layer and its specific resistivity. In practice CL expressed in volts should be preferably  $\geq 30$  d, where d is the thickness in  $\mu$ m of the charge transport layer.

In the accompanying FIGS. 1 to 21 sensitometric curves are given with in the abscissa logarithmic values of exposure dose at 540 nm [ $\log E = \log I \cdot t$ ] expressed in mJ/m<sup>2</sup> and in the ordinate voltage values [V] measured on the charged recording layer during the exposure using increasing exposure doses at constant exposure time.

The following examples further illustrate the present invention. All parts, ratios and percentages are by weight unless otherwise stated.

#### COMPARATIVE EXAMPLES 1 TO 3

In the photoconductive recording materials of COMPARATIVE EXAMPLES 1 to 3 a 100  $\mu$ m thick polyester layer precoated with a vacuum-deposited conductive layer of aluminium was doctor-blade coated with a dispersion of N,N'dimethyl perylimide C.I. Pigment

Red 189, C.I. No 71130 (represented as PIM in Table 1) containing the charge transport material 2,5-bis(4-N,N-

factor of 3.16 difference in exposure. The results are given in Table 1.

TABLE 1

| Comparative Example no. | PIM conc. [wt %] | OXA conc. [wt %] | P1 conc. [wt %] | P2 conc. [wt %] | Layer thickness [μm] | CL [V] | % discharge for $I_{540t}$ of 38 mJ/m <sup>2</sup> | % discharge between $I_{540t}$ 's of 12 and 38 mJ/m <sup>2</sup> |
|-------------------------|------------------|------------------|-----------------|-----------------|----------------------|--------|----------------------------------------------------|------------------------------------------------------------------|
| 1                       | 15               | 10               | 67.5            | 7.5             | 13                   | -281   | 12.8*                                              | 28.1                                                             |
| 2                       | 15               | 8                | 69.3            | 7.7             | 13                   | -232   | 0*                                                 | 19.4                                                             |
| 3                       | 15               | 5                | 72              | 8               | 13                   | -281   | 5.7*                                               | 17.8                                                             |

\*CL fluctuation during measurement.

diethylaminophenyl)oxidiazole-1,3,4 (represented as OXA in Table 1). In said Table 1 also the concentrations (conc.) and layer thicknesses in μm are given.

Said dispersions were prepared by mixing for 72 hours in a ball mill N,N'dimethylperylimide, an aromatic polycarbonate MAKROLON CD 2000 (registered trade mark), indicated in Table 1 as P1 in the weight percentages given in said Table 1 in dichloromethane at a solids concentration of 16.2% by weight and subsequently adding 2,5-bis(4-N,N-diethylaminophenyl)oxidiazole-1,3,4 and a polyester adhesion-promoting additive DYNAPOL L206 (registered trade mark), indicated in Table 1 as P2 in the weight percentages given in said Table 1 with additional dichloromethane and mixing for a further 30 minutes. The dispersion was then cast without further dilution with dichloromethane and the resulting layer dried for 16 hours at 50° C.

COMPARATIVE EXAMPLE 1 has the same N,N'dimethylperylimide and 2,5-bis(4-N,N-diethylaminophenyl)oxidiazole-1,3,4 concentrations as in EXAMPLE 1 of published EP-A 161 648 corresponding with U.S. Pat. No. 4,668,600 and binder types described as preferred in said documents.

The characteristics of the thus obtained photosensitive materials were determined as described above. The sensitivity to monochromatic 540 nm light exposure is expressed as the % discharge at an exposure ( $I_{540t}$ ) of 38 mJ/m<sup>2</sup> and the steepness of the discharge exposure dependence is expressed as the % discharge observed between exposures ( $I_{540t}$ ) of 12 mJ/m<sup>2</sup> and 38 mJ/m<sup>2</sup>, a

#### EXAMPLES 1 to 22 and COMPARATIVE EXAMPLES 4 to 13

In the production of the photosensitive recording materials a 100 μm thick polyester film precoated with a vacuum-deposited conductive layer of aluminium was doctor-blade coated with a dispersion of charge generating pigment containing charge transport material, the respective compositions being given in Table 2, to thicknesses in μm also given in Table 2.

Said dispersion was prepared by mixing for 15 minutes in a pearl mill 4,10-dibromoanthrone (DBA), 1,2-bis(1,2-dihydro-2,2,4-trimethylquinolin-1-yl)ethane (Bisflectol), a polyester adhesion-promoting additive DYNAPOL L206 (registered trade mark), indicated in Table 2 as P2, and an aromatic polycarbonate MAKROLON CD 2000 (registered trade mark), indicated in Table 2 as P1 in the weight percentages given in said Table 2 using dichloromethane as coating solvent (17.16 g/g DBA). The dispersion was cast without further dilution with dichloromethane and the resulting layer dried for 15 hours at 50° C.

The characteristics of the thus obtained photosensitive recording materials were determined as described above. The sensitivity to monochromatic 540 nm light exposure is expressed as the % discharge at an exposure ( $I_{540t}$ ) of 36.6 mJ/m<sup>2</sup> and the steepness of the discharge exposure dependence is expressed as the % discharge observed between exposures ( $I_{540t}$ ) of 11.6 mJ/m<sup>2</sup> and 36.6 mJ/m<sup>2</sup>, a factor of 3.16 difference in exposure. The results are given in Table 2.

TABLE 2

| Example no. | DBA conc. [wt %] | Bisflectol conc. [wt %] | P1 conc. [wt %] | P2 conc. [wt %] | layer thickness [μm] | CL [V] | % discharge for $I_{540t} = 36.6$ mJ/m <sup>2</sup> | % discharge between $I_{540t}$ 's of 11.6 and 36.6 mJ/m <sup>2</sup> |
|-------------|------------------|-------------------------|-----------------|-----------------|----------------------|--------|-----------------------------------------------------|----------------------------------------------------------------------|
| 1           | 30               | 5                       | 58.5            | 6.5             | 12                   | -730   | 90.0                                                | 81.1                                                                 |
| 2           | 30               | 10                      | 54              | 6.0             | 11                   | -679   | 94.7                                                | 79.4                                                                 |
| 3           | 30               | 20                      | 45              | 5.0             | 10                   | -625   | 97.4                                                | 71.0                                                                 |
| 4           | 30               | 30                      | 36              | 4.0             | 10                   | -574   | 93.0                                                | 56.4                                                                 |
| 5           | 30               | 40                      | 27              | 3.0             | 13                   | -666   | 72.7                                                | 40.0                                                                 |
| 6           | 25               | 5                       | 63              | 7.0             | 11                   | -704   | 79.0                                                | 68.9                                                                 |
| 7           | 25               | 10                      | 58.5            | 6.5             | 10                   | -758   | 95.6                                                | 79.0                                                                 |
| 8           | 25               | 15                      | 54              | 6.0             | 10                   | -667   | 96.0                                                | 75.2                                                                 |
| 9           | 25               | 25                      | 45              | 5.0             | 11                   | -640   | 95.8                                                | 70.9                                                                 |
| 10          | 25               | 30                      | 40.5            | 4.5             | 8                    | -524   | 96.6                                                | 60.9                                                                 |
| 11          | 25               | 40                      | 31.5            | 3.5             | 10                   | -515   | 92.6                                                | 53.0                                                                 |
| 12          | 20               | 10                      | 63              | 7.0             | 12                   | -683   | 89.5                                                | 72.2                                                                 |
| 13          | 20               | 15                      | 58.5            | 6.5             | 12                   | -768   | 95.1                                                | 75.8                                                                 |
| 14          | 20               | 20                      | 54              | 6.0             | 12                   | -718   | 93.6                                                | 73.7                                                                 |
| 15          | 20               | 30                      | 45              | 5.0             | 11                   | -636   | 90.3                                                | 63.1                                                                 |
| 16          | 20               | 40                      | 36              | 4.0             | 13                   | -641   | 88.6                                                | 58.5                                                                 |
| 17          | 15               | 10                      | 67.5            | 7.5             | 12                   | -703   | 81.8                                                | 66.1                                                                 |
| 18          | 15               | 15                      | 63              | 7.0             | 12                   | -784   | 72.4                                                | 55.4                                                                 |
| 19          | 15               | 20                      | 58.5            | 6.5             | 11                   | -697   | 66.1                                                | 44.6                                                                 |
| 20          | 16               | 24                      | 54              | 6.0             | 10                   | -617   | 82.2                                                | 54.5                                                                 |
| 21          | 15               | 30                      | 49.5            | 5.5             | 8                    | -606   | 81.2                                                | 48.2                                                                 |
| 22          | 15               | 40                      | 40.5            | 4.5             | 8                    | -572   | 91.6                                                | 49.3                                                                 |

TABLE 2-continued

| Comparative example no. | DBA conc. [wt %] | Bis-flectol conc. [wt %] | P1 conc. [wt %] | P2 conc. [wt %] | layer thickness [μm] | CL [V] | % discharge for $I_{540t} = 36.6 \text{ mJ/m}^2$ | % discharge between $I_{540t}$ 's of 11.6 and 36.6 $\text{mJ/m}^2$ |
|-------------------------|------------------|--------------------------|-----------------|-----------------|----------------------|--------|--------------------------------------------------|--------------------------------------------------------------------|
| 4                       | 40               | 0                        | 54.0            | 6.0             | 12                   | -849   | 4.9                                              | 2.8                                                                |
| 5                       | 25               | 0                        | 67.5            | 7.5             | 12                   | -817   | 2.8                                              | 2.1                                                                |
| 6                       | 20               | 50                       | 27.0            | 3.0             | 11                   | -654   | 69.7                                             | 36.4                                                               |
| 7                       | 15               | 50                       | 31.5            | 3.5             | 10                   | -638   | 75.7                                             | 37.6                                                               |
| 8                       | 10               | 30                       | 54.0            | 6.0             | 12                   | -765   | 64.3                                             | 31.9                                                               |
| 9                       | 10               | 40                       | 45.0            | 5.0             | 12                   | -766   | 66.2                                             | 31.6                                                               |
| 10                      | 10               | 50                       | 36.0            | 4.0             | 13                   | -742   | 72.2                                             | 32.9                                                               |
| 11                      | 5                | 30                       | 58.5            | 6.5             | 22                   | -1000  | 48.4                                             | 24.1                                                               |
| 12                      | 5                | 40                       | 49.5            | 5.5             | 22                   | -1024  | 58.6                                             | 25.9                                                               |
| 13                      | 5                | 50                       | 40.5            | 4.5             | 22                   | -1030  | 68.7                                             | 29.4                                                               |

A sensitometric measurement was carried out on the photosensitive recording material of comparative Example 9 using the refined sensitometric measurement techniques described above. The resulting sensitometric curve is shown in FIG. 1 with exposures required for 10% and 90% discharges differing by a factor of greater than 10.

#### EXAMPLES 23 to 27 and COMPARATIVE EXAMPLES 14 and 15

The photosensitive recording materials of EXAMPLES 23 to 27 and COMPARATIVE EXAMPLES 14 and 15 were produced as described for EXAMPLES 1 to 22 with the compositions and layer thicknesses given together with the % discharges at an exposure ( $I_{540t}$ ) of 36.6  $\text{mJ/m}^2$  and the % discharges observed between exposures ( $I_{540t}$ ) of 11.6  $\text{mJ/m}^2$  and 36.6  $\text{mJ/m}^2$  are given in Table 3.

TABLE 3

| Example no.         | DBA conc. [wt %] | Bis-flectol conc. [wt %] | P1 conc. [wt %] | P2 conc. [wt %] | layer thickness [μm] | CL [V] | % discharge for $I_{540t} = 36.6 \text{ mJ/m}^2$ | % discharge between $I_{540t}$ 's of 11.6 and 36.6 $\text{mJ/m}^2$ |
|---------------------|------------------|--------------------------|-----------------|-----------------|----------------------|--------|--------------------------------------------------|--------------------------------------------------------------------|
| 23                  | 25               | 10                       | 58.5            | 6.5             | 4                    | -486   | 78.8                                             | 60.3                                                               |
| 24                  | 25               | 10                       | 58.5            | 6.5             | 6                    | -591   | 87.3                                             | 71.9                                                               |
| 7                   | 25               | 10                       | 58.5            | 6.5             | 10                   | -758   | 95.6                                             | 79.0                                                               |
| 25                  | 25               | 10                       | 58.5            | 6.5             | 12                   | -730   | 93.8                                             | 77.7                                                               |
| 26                  | 25               | 10                       | 58.5            | 6.5             | 15                   | -826   | 96.0                                             | 73.5                                                               |
| 27                  | 25               | 10                       | 58.5            | 6.5             | 18                   | -997   | 94.2                                             | 71.7                                                               |
| Comparative example |                  |                          |                 |                 |                      |        |                                                  |                                                                    |
| 14                  | 25               | 10                       | 58.5            | 6.5             | 2.5                  | -300   | 68.3                                             | 49.3                                                               |
| 15                  | 25               | 10                       | 58.5            | 6.5             | 27                   | -981   | 81.0                                             | 55.7                                                               |

#### EXAMPLE 28

The photosensitive recording material of EXAMPLE 28 was produced as described for EXAMPLE 7 except that 1,2-bis(6-ethoxy-1,2-dihydro-2,2,4-trimethylquinolin-1-yl)ethane was used as the charge transport material instead of 1,2-bis(1,2-dihydro-2,2,4-trimethylquinolin-1-yl)ethane. The layer thickness was 12  $\mu\text{m}$ . This photosensitive recording material exhibited 89.8% discharge upon  $I_{540t}$  exposure of 36.6  $\text{mJ/m}^2$  and 77.2% discharge between  $I_{540t}$  exposures of 11.6  $\text{mJ/m}^2$  and 36.6  $\text{mJ/m}^2$ .

#### EXAMPLE 29

The photosensitive recording material of EXAMPLE 29 was produced as described for EXAMPLE 7

except that N,N'-bis(3,5-xylyl) perylimide C.I. Pigment Red 149 and C.I. 71 137 was used as the sensitizing pigment instead of 4,10-dibromoanthanthrone [C.I. Pigment Red 168 and C.I. 59 300]. The layer thickness was 13  $\mu\text{m}$ . This photosensitive recording material exhibited 93.3% discharge upon  $I_{540t}$  exposure of 36.6  $\text{mJ/m}^2$  and 90.6% discharge between  $I_{540t}$  exposures of 11.6  $\text{mJ/m}^2$  and 36.6  $\text{mJ/m}^2$ . The sensitometric curve obtained using the refined sensitometric measurement technique described above is shown in FIG. 2.

#### EXAMPLE 30

The photosensitive recording material of EXAMPLE 30 was produced as described for EXAMPLE 7 except that N,N'-bis(4-ethoxyphenyl)perylimide C.I. Pigment Red 123 and C.I. 71 145 was used as the sensitizing pigment instead of 4,10-dibromoanthanthrone C.I. Pigment Red 168 and C.I. 59 300. The layer thick-

ness was 13  $\mu\text{m}$ . This photosensitive recording material exhibited 19.2% discharge upon  $I_{540t}$  exposure of 36.6  $\text{mJ/m}^2$  and 64.4% discharge between  $I_{540t}$  exposures of 36.6  $\text{mJ/m}^2$  and 116  $\text{mJ/m}^2$ .

#### EXAMPLE 31

The photosensitive recording material of EXAMPLE 31 was produced as described for EXAMPLE 7 except that the binder resin consisted of 100% of DYNAPOL L206 (registered trade mark) instead of a mixture of DYNAPOL L206 (registered trade mark) and an aromatic polycarbonate MAKROLON CD 2000 (registered trade mark). The layer thickness was 11  $\mu\text{m}$ . This photosensitive recording material exhibited 94.3% discharge upon  $I_{540t}$  exposure of 36.6  $\text{mJ/m}^2$  and

75.7% discharge between  $I_{540t}$  exposures of 11.6 mJ/m<sup>2</sup> and 36.6 mJ/m<sup>2</sup>.

### EXAMPLE 32

The photosensitive recording material of EXAMPLE 32 was produced as described for EXAMPLE 7 except that the 100  $\mu\text{m}$  thick polyester film was precoated with a vacuum-deposited conductive layer of aluminium and was doctor blade coated with a 1% solution of  $\gamma$ -aminopropyltriethoxy silane in aqueous methanol. The solvent was evaporated and the layer cured at 100° C. for 30 minutes prior to the coating of the photoconductive recording layer. The photoconductive layer had a thickness of 12  $\mu\text{m}$  and exhibited 93.8% discharge upon  $I_{540t}$  exposure of 36.6 mJ/m<sup>2</sup> and 77.7% discharge between  $I_{540t}$  exposures of 11.6 mJ/m<sup>2</sup>.

### EXAMPLE 33

The photosensitive recording material of EXAMPLE 33 was produced as described for EXAMPLE 32 except that the binder resin in the photoconductive layer was 100% aromatic polycarbonate MAKROLON CD 2000 (registered trade mark) instead of a mixture of DYNAPOL L206 (registered trade mark) and MAKROLON CD 2000 (registered trade mark). The layer thickness was 12  $\mu\text{m}$ . This photosensitive recording material exhibited 85.3% discharge upon  $I_{540t}$  exposure of 36.6 mJ/m<sup>2</sup> and 63.3% discharge between  $I_{540t}$  exposures of 11.6 mJ/m<sup>2</sup> and 36.6 mJ/m<sup>2</sup>.

### COMPARATIVE EXAMPLE 16

A double layer functionally separated photosensitive recording material was produced by first doctor blade-coating a 100  $\mu\text{m}$  thick polyester film precoated with a vacuum-deposited conductive layer of aluminium with a 1% solution of  $\gamma$ -aminopropyltriethoxy silane in aqueous methanol. After solvent evaporation and curing at 100° C. for 30 minutes, the thus obtained adhesion/-blocking layer was doctor blade-coated with a dispersion of charge generating pigment to a thickness of 0.6

5   
 10   
 15   
 20   
 25   
 30   
 35   
 40   
 45   
 50   
 55   
 60   
 65   
 70   
 75   
 80   
 85   
 90   
 95   
 100   
 105   
 110   
 115   
 120   
 125   
 130   
 135   
 140   
 145   
 150   
 155   
 160   
 165   
 170   
 175   
 180   
 185   
 190   
 195   
 200   
 205   
 210   
 215   
 220   
 225   
 230   
 235   
 240   
 245   
 250   
 255   
 260   
 265   
 270   
 275   
 280   
 285   
 290   
 295   
 300   
 305   
 310   
 315   
 320   
 325   
 330   
 335   
 340   
 345   
 350   
 355   
 360   
 365   
 370   
 375   
 380   
 385   
 390   
 395   
 400   
 405   
 410   
 415   
 420   
 425   
 430   
 435   
 440   
 445   
 450   
 455   
 460   
 465   
 470   
 475   
 480   
 485   
 490   
 495   
 500   
 505   
 510   
 515   
 520   
 525   
 530   
 535   
 540   
 545   
 550   
 555   
 560   
 565   
 570   
 575   
 580   
 585   
 590   
 595   
 600   
 605   
 610   
 615   
 620   
 625   
 630   
 635   
 640   
 645   
 650   
 655   
 660   
 665   
 670   
 675   
 680   
 685   
 690   
 695   
 700   
 705   
 710   
 715   
 720   
 725   
 730   
 735   
 740   
 745   
 750   
 755   
 760   
 765   
 770   
 775   
 780   
 785   
 790   
 795   
 800   
 805   
 810   
 815   
 820   
 825   
 830   
 835   
 840   
 845   
 850   
 855   
 860   
 865   
 870   
 875   
 880   
 885   
 890   
 895   
 900   
 905   
 910   
 915   
 920   
 925   
 930   
 935   
 940   
 945   
 950   
 955   
 960   
 965   
 970   
 975   
 980   
 985   
 990   
 995   
 1000   
 1005   
 1010   
 1015   
 1020   
 1025   
 1030   
 1035   
 1040   
 1045   
 1050   
 1055   
 1060   
 1065   
 1070   
 1075   
 1080   
 1085   
 1090   
 1095   
 1100   
 1105   
 1110   
 1115   
 1120   
 1125   
 1130   
 1135   
 1140   
 1145   
 1150   
 1155   
 1160   
 1165   
 1170   
 1175   
 1180   
 1185   
 1190   
 1195   
 1200   
 1205   
 1210   
 1215   
 1220   
 1225   
 1230   
 1235   
 1240   
 1245   
 1250   
 1255   
 1260   
 1265   
 1270   
 1275   
 1280   
 1285   
 1290   
 1295   
 1300   
 1305   
 1310   
 1315   
 1320   
 1325   
 1330   
 1335   
 1340   
 1345   
 1350   
 1355   
 1360   
 1365   
 1370   
 1375   
 1380   
 1385   
 1390   
 1395   
 1400   
 1405   
 1410   
 1415   
 1420   
 1425   
 1430   
 1435   
 1440   
 1445   
 1450   
 1455   
 1460   
 1465   
 1470   
 1475   
 1480   
 1485   
 1490   
 1495   
 1500   
 1505   
 1510   
 1515   
 1520   
 1525   
 1530   
 1535   
 1540   
 1545   
 1550   
 1555   
 1560   
 1565   
 1570   
 1575   
 1580   
 1585   
 1590   
 1595   
 1600   
 1605   
 1610   
 1615   
 1620   
 1625   
 1630   
 1635   
 1640   
 1645   
 1650   
 1655   
 1660   
 1665   
 1670   
 1675   
 1680   
 1685   
 1690   
 1695   
 1700   
 1705   
 1710   
 1715   
 1720   
 1725   
 1730   
 1735   
 1740   
 1745   
 1750   
 1755   
 1760   
 1765   
 1770   
 1775   
 1780   
 1785   
 1790   
 1795   
 1800   
 1805   
 1810   
 1815   
 1820   
 1825   
 1830   
 1835   
 1840   
 1845   
 1850   
 1855   
 1860   
 1865   
 1870   
 1875   
 1880   
 1885   
 1890   
 1895   
 1900   
 1905   
 1910   
 1915   
 1920   
 1925   
 1930   
 1935   
 1940   
 1945   
 1950   
 1955   
 1960   
 1965   
 1970   
 1975   
 1980   
 1985   
 1990   
 1995   
 2000   
 2005   
 2010   
 2015   
 2020   
 2025   
 2030   
 2035   
 2040   
 2045   
 2050   
 2055   
 2060   
 2065   
 2070   
 2075   
 2080   
 2085   
 2090   
 2095   
 2100   
 2105   
 2110   
 2115   
 2120   
 2125   
 2130   
 2135   
 2140   
 2145   
 2150   
 2155   
 2160   
 2165   
 2170   
 2175   
 2180   
 2185   
 2190   
 2195   
 2200   
 2205   
 2210   
 2215   
 2220   
 2225   
 2230   
 2235   
 2240   
 2245   
 2250   
 2255   
 2260   
 2265   
 2270   
 2275   
 2280   
 2285   
 2290   
 2295   
 2300   
 2305   
 2310   
 2315   
 2320   
 2325   
 2330   
 2335   
 2340   
 2345   
 2350   
 2355   
 2360   
 2365   
 2370   
 2375   
 2380   
 2385   
 2390   
 2395   
 2400   
 2405   
 2410   
 2415   
 2420   
 2425   
 2430   
 2435   
 2440   
 2445   
 2450   
 2455   
 2460   
 2465   
 2470   
 2475   
 2480   
 2485   
 2490   
 2495   
 2500   
 2505   
 2510   
 2515   
 2520   
 2525   
 2530   
 2535   
 2540   
 2545   
 2550   
 2555   
 2560   
 2565   
 2570   
 2575   
 2580   
 2585   
 2590   
 2595   
 2600   
 2605   
 2610   
 2615   
 2620   
 2625   
 2630   
 2635   
 2640   
 2645   
 2650   
 2655   
 2660   
 2665   
 2670   
 2675   
 2680   
 2685   
 2690   
 2695   
 2700   
 2705   
 2710   
 2715   
 2720   
 2725   
 2730   
 2735   
 2740   
 2745   
 2750   
 2755   
 2760   
 2765   
 2770   
 2775   
 2780   
 2785   
 2790   
 2795   
 2800   
 2805   
 2810   
 2815   
 2820   
 2825   
 2830   
 2835   
 2840   
 2845   
 2850   
 2855   
 2860   
 2865   
 2870   
 2875   
 2880   
 2885   
 2890   
 2895   
 2900   
 2905   
 2910   
 2915   
 2920   
 2925   
 2930   
 2935   
 2940   
 2945   
 2950   
 2955   
 2960   
 2965   
 2970   
 2975   
 2980   
 2985   
 2990   
 2995   
 3000   
 3005   
 3010   
 3015   
 3020   
 3025   
 3030   
 3035   
 3040   
 3045   
 3050   
 3055   
 3060   
 3065   
 3070   
 3075   
 3080   
 3085   
 3090   
 3095   
 3100   
 3105   
 3110   
 3115   
 3120   
 3125   
 3130   
 3135   
 3140   
 3145   
 3150   
 3155   
 3160   
 3165   
 3170   
 3175   
 3180   
 3185   
 3190   
 3195   
 3200   
 3205   
 3210   
 3215   
 3220   
 3225   
 3230   
 3235   
 3240   
 3245   
 3250   
 3255   
 3260   
 3265   
 3270   
 3275   
 3280   
 3285   
 3290   
 3295   
 3300   
 3305   
 3310   
 3315   
 3320   
 3325   
 3330   
 3335   
 3340   
 3345   
 3350   
 3355   
 3360   
 3365   
 3370   
 3375   
 3380   
 3385   
 3390   
 3395   
 3400   
 3405   
 3410   
 3415   
 3420   
 3425   
 3430   
 3435   
 3440   
 3445   
 3450   
 3455   
 3460   
 3465   
 3470   
 3475   
 3480   
 3485   
 3490   
 3495   
 3500   
 3505   
 3510   
 3515   
 3520   
 3525   
 3530   
 3535   
 3540   
 3545   
 3550   
 3555   
 3560   
 3565   
 3570   
 3575   
 3580   
 3585   
 3590   
 3595   
 3600   
 3605   
 3610   
 3615   
 3620   
 3625   
 3630   
 3635   
 3640   
 3645   
 3650   
 3655   
 3660   
 3665   
 3670   
 3675   
 3680   
 3685   
 3690   
 3695   
 3700   
 3705   
 3710   
 3715   
 3720   
 3725   
 3730   
 3735   
 3740   
 3745   
 3750   
 3755   
 3760   
 3765   
 3770   
 3775   
 3780   
 3785   
 3790   
 3795   
 3800   
 3805   
 3810   
 3815   
 3820   
 3825   
 3830   
 3835   
 3840   
 3845   
 3850   
 3855   
 3860   
 3865   
 3870   
 3875   
 3880   
 3885   
 3890   
 3895   
 3900   
 3905   
 3910   
 3915   
 3920   
 3925   
 3930   
 3935   
 3940   
 3945   
 3950   
 3955   
 3960   
 3965   
 3970   
 3975   
 3980   
 3985   
 3990   
 3995   
 4000   
 4005   
 4010   
 4015   
 4020   
 4025   
 4030   
 4035   
 4040   
 4045   
 4050   
 4055   
 4060   
 4065   
 4070   
 4075   
 4080   
 4085   
 4090   
 4095   
 4100   
 4105   
 4110   
 4115   
 4120   
 4125   
 4130   
 4135   
 4140   
 4145   
 4150   
 4155   
 4160   
 4165   
 4170   
 4175   
 4180   
 4185   
 4190   
 4195   
 4200   
 4205   
 4210   
 4215   
 4220   
 4225   
 4230   
 4235   
 4240   
 4245   
 4250   
 4255   
 4260   
 4265   
 4270   
 4275   
 4280   
 4285   
 4290   
 4295   
 4300   
 4305   
 4310   
 4315   
 4320   
 4325   
 4330   
 4335   
 4340   
 4345   
 4350   
 4355   
 4360   
 4365   
 4370   
 4375   
 4380   
 4385   
 4390   
 4395   
 4400   
 4405   
 4410   
 4415   
 4420   
 4425   
 4430   
 4435   
 4440   
 4445   
 4450   
 4455   
 4460   
 4465   
 4470   
 4475   
 4480   
 4485   
 4490   
 4495   
 4500   
 4505   
 4510   
 4515   
 4520   
 4525   
 4530   
 4535   
 4540   
 4545   
 4550   
 4555   
 4560   
 4565   
 4570   
 4575   
 4580   
 4585   
 4590   
 4595   
 4600   
 4605   
 4610   
 4615   
 4620   
 4625   
 4630   
 4635   
 4640   
 4645   
 4650   
 4655   
 4660   
 4665   
 4670   
 4675   
 4680   
 4685   
 4690   
 4695   
 4700   
 4705   
 4710   
 4715   
 4720   
 4725   
 4730   
 4735   
 4740   
 4745   
 4750   
 4755   
 4760   
 4765   
 4770   
 4775   
 4780   
 4785   
 4790   
 4795   
 4800   
 4805   
 4810   
 4815   
 4820   
 4825   
 4830   
 4835   
 4840   
 4845   
 4850   
 4855   
 4860   
 4865   
 4870   
 4875   
 4880   
 4885   
 4890   
 4895   
 4900   
 4905   
 4910   
 4915   
 4920   
 4925   
 4930   
 4935   
 4940   
 4945   
 4950   
 4955   
 4960   
 4965   
 4970   
 4975   
 4980   
 4985   
 4990   
 4995   
 5000   
 5005   
 5010   
 5015   
 5020   
 5025   
 5030   
 5035   
 5040   
 5045   
 5050   
 5055   
 5060   
 5065   
 5070   
 5075   
 5080   
 5085   
 5090   
 5095   
 5100   
 5105   
 5110   
 5115   
 5120   
 5125   
 5130   
 5135   
 5140   
 5145   
 5150   
 5155   
 5160   
 5165   
 5170   
 5175   
 5180   
 5185   
 5190   
 5195   
 5200   
 5205   
 5210   
 5215   
 5220   
 5225   
 5230   
 5235   
 5240   
 5245   
 5250   
 5255   
 5260   
 5265   
 5270   
 5275   
 5280   
 5285   
 5290   
 5295   
 5300   
 5305   
 5310   
 5315   
 5320   
 5325   
 5330   
 5335   
 5340   
 5345   
 5350   
 5355   
 5360   
 5365   
 5370   
 5375   
 5380   
 5385   
 5390   
 5395   
 5400   
 5405   
 5410   
 5415   
 5420   
 5425   
 5430   
 5435   
 5440   
 5445   
 5450   
 5455   
 5460   
 5465   
 5470   
 5475   
 5480   
 5485   
 5490   
 5495   
 5500   
 5505   
 5510   
 5515   
 5520   
 5525   
 5530   
 5535   
 5540   
 5545   
 5550   
 5555   
 5560   
 5565   
 5570   
 5575   
 5580   
 5585   
 5590   
 5595   
 5600   
 5605   
 5610   
 5615   
 5620   
 5625   
 5630   
 5635   
 5640   
 5645   
 5650   
 5655   
 5660   
 5665   
 5670   
 5675   
 5680   
 5685   
 5690   
 5695   
 5700   
 5705   
 5710   
 5715   
 5720   
 5725   
 5730   
 5735   
 5740   
 5745   
 5750   
 5755   
 5760   
 5765   
 5770   
 5775   
 5780   
 5785   
 5790   
 5795   
 5800   
 5805   
 5810   
 5815   
 5820   
 5825   
 5830   
 5835   
 5840   
 5845   
 5850   
 5855   
 5860   
 5865   
 5870   
 5875   
 5880   
 5885   
 5890   
 5895   
 5900   
 5905   
 5910   
 5915   
 5920   
 5925   
 5930   
 5935   
 5940   
 5945   
 5950   
 5955   
 5960   
 5965   
 5970   
 5975   
 5980   
 5985   
 5990   
 5995   
 6000   
 6005   
 6010   
 6015   
 6020   
 6025   
 6030   
 6035   
 6040   
 6045   
 6050   
 6055   
 6060   
 6065   
 6070   
 6075   
 6080   
 6085   
 6090   
 6095   
 6100   
 6105   
 6110   
 6115   
 6120   
 6125   
 6130   
 6135   
 6140   
 6145   
 6150   
 6155   
 6160   
 6165   
 6170   
 6175   
 6180   
 6185   
 6190   
 6195   
 6200   
 6205   
 6210   
 6215   
 6220   
 6225   
 6230   
 6235   
 6240   
 6245   
 6250   
 6255   
 6260   
 6265   
 6270   
 6275   
 6280   
 6285   
 6290   
 6295   
 6300   
 6305   
 6310   
 6315   
 6320   
 6325   
 6330   
 6335   
 6340   
 6345   
 6350   
 6355   
 6360   
 6365   
 6370   
 6375   
 6380   
 6385   
 6390   
 6395   
 6400   
 6405   
 6410   
 6415   
 6420   
 6425   
 6430   
 6435   
 6440   
 6445   
 6450   
 6455   
 6460   
 6465   
 6470   
 6475   
 6480   
 6485   
 6490   
 6495   
 6500   
 6505   
 6510   
 6515   
 6520   
 6525   
 6530   
 6535   
 6540   
 6545   
 6550   
 6555   
 6560   
 6565   
 6570   
 6575   
 6580   
 6585   
 6590   
 6595   
 6600   
 6605   
 6610   
 6615   
 6620   
 6625   
 6630   
 6635   
 6640   
 6645   
 6650   
 6655   
 6660   
 6665 <

## EXAMPLES 37 TO 45 AND COMPARATIVE EXAMPLES 18 AND 19

The photosensitive recording materials of EXAMPLES 37 to 45 and of COMPARATIVE EXAMPLES 18 and 19 were produced as described for EXAMPLE 38 except that the concentration of 1,2-bis-(dihydro-2,2,4-trimethyl-quinolin-1-yl)ethane (called herein Bis-flectol) varied from 50 to 0 wt % as given in Tables 5A and 5B and the concentrations of binders varied appropriately as also given in Tables 5A and 5B together with the layer thicknesses.

The characteristics of the thus obtained photosensitive recording materials were determined as described above and are given in Tables 5A and 5B. The sensitivity to monochromatic 540 nm light exposure is expressed as the % discharge at an exposure ( $I_{540t}$ ) of 36.6 mJ/m<sup>2</sup> and the steepness of the discharge-exposure dependence is expressed as the % discharge observed between exposures ( $I_{540t}$ ) of 11.6 mJ/m<sup>2</sup> and 36.6 mJ/m<sup>2</sup> (see Table 5A), or 36.6 mJ/m<sup>2</sup> and 116 mJ/m<sup>2</sup> or 76 mJ/m<sup>2</sup> and 240 mJ/m<sup>2</sup> (see Table 5B) depending upon the sensitivity of the photosensitive recording material.

TABLE 5A

|                                | DBA conc.<br>[wt %] | Bis-flectol conc.<br>[wt %] | P1 conc.<br>[wt %] | P2 conc.<br>[wt %] | layer thickness<br>[μm] | CL<br>[V] | % discharge for $I_{540t}$ = 36.6 mJ/m <sup>2</sup> | % discharge between $I_{540t}$ 's of 11.6 and 36.6 mJ/m <sup>2</sup> |
|--------------------------------|---------------------|-----------------------------|--------------------|--------------------|-------------------------|-----------|-----------------------------------------------------|----------------------------------------------------------------------|
| <b>Example No.</b>             |                     |                             |                    |                    |                         |           |                                                     |                                                                      |
| 37                             | 25                  | 40                          | 31.5               | 3.5                | 13                      | -624      | 68.3                                                | 45.0                                                                 |
| 38                             | 25                  | 30                          | 40.5               | 4.5                | 11                      | -598      | 75.9                                                | 53.8                                                                 |
| 39                             | 25                  | 10                          | 58.5               | 6.5                | 17                      | -916      | 95.5                                                | 83.6                                                                 |
| 40                             | 25                  | 5                           | 63.0               | 7.0                | 16                      | -823      | 91.6                                                | 85.4                                                                 |
| 41                             | 25                  | 3                           | 64.8               | 7.2                | 17                      | -844      | 91.1                                                | 88.0                                                                 |
| 42                             | 25                  | 1                           | 66.6               | 7.4                | 15                      | -911      | 86.2                                                | 83.6                                                                 |
| 43                             | 25                  | 0.3                         | 67.23              | 7.47               | 11                      | -996      | 4.8                                                 | —                                                                    |
| 44                             | 25                  | 0.1                         | 67.41              | 7.49               | 12                      | -1034     | 3.3                                                 | —                                                                    |
| 45                             | 25                  | 0.03                        | 67.473             | 7.497              | 13                      | -1012     | 1.2                                                 | —                                                                    |
| <b>Comparative Example No.</b> |                     |                             |                    |                    |                         |           |                                                     |                                                                      |
| 18                             | 25                  | 0                           | 67.5               | 7.5                | 12                      | -980      | 2.3                                                 | —                                                                    |
| 19                             | 25                  | 50                          | 22.5               | 2.5                | 17                      | -648      | 65.6                                                | 40.4                                                                 |

TABLE 5B

|                                | DBA conc.<br>[wt %] | Bis-flectol conc.<br>[wt %] | P1 conc.<br>[wt %] | P2 conc.<br>[wt %] | layer thickness<br>[μm] | CL<br>[V] | % discharge between $I_{540t}$ 's of 36.6 and 116 mJ/m <sup>2</sup> | % discharge between $I_{540t}$ 's of 76 and 240 mJ/m <sup>2</sup> |
|--------------------------------|---------------------|-----------------------------|--------------------|--------------------|-------------------------|-----------|---------------------------------------------------------------------|-------------------------------------------------------------------|
| <b>Example No.</b>             |                     |                             |                    |                    |                         |           |                                                                     |                                                                   |
| 43                             | 25                  | 0.3                         | 67.23              | 7.47               | 11                      | -996      | 71.6                                                                | 75.2                                                              |
| 44                             | 25                  | 0.1                         | 67.41              | 7.49               | 12                      | -1034     | —                                                                   | 75.5                                                              |
| 45                             | 25                  | 0.03                        | 67.473             | 7.497              | 13                      | -1012     | —                                                                   | 64.7                                                              |
| <b>Comparative Example No.</b> |                     |                             |                    |                    |                         |           |                                                                     |                                                                   |
| 18                             | 25                  | 0                           | 67.5               | 7.5                | 12                      | -980      | —                                                                   | 30.6                                                              |

TABLE 6A

|                    | DBA conc.<br>[wt %] | Bis-flectol conc.<br>[wt %] | P1 conc.<br>[wt %] | P2 conc.<br>[wt %] | layer thickness<br>[μm] | CL<br>[V] | % discharge for $I_{540t}$ = 36.6 mJ/m <sup>2</sup> | % discharge between $I_{540t}$ 's of 36.6 and 11.6 mJ/m <sup>2</sup> |
|--------------------|---------------------|-----------------------------|--------------------|--------------------|-------------------------|-----------|-----------------------------------------------------|----------------------------------------------------------------------|
| <b>Example No.</b> |                     |                             |                    |                    |                         |           |                                                     |                                                                      |
| 1                  | 30                  | 5                           | 58.5               | 6.5                | 12                      | -730      | 90.0                                                | —                                                                    |
| 46                 | 40                  | 5                           | 49.5               | 5.5                | 15                      | -639      | 95.1                                                | 87.5                                                                 |
| 47                 | 50                  | 5                           | 40.5               | 4.5                | 15                      | -662      | 97.7                                                | 82.0                                                                 |

## EXAMPLES 46 TO 49 AND COMPARATIVE EXAMPLE 20

The photosensitive recording materials of EXAMPLES 46 to 49 and of COMPARATIVE EXAMPLE 20 were produced as described for EXAMPLE 1 except that the concentration of 4,10-dibromo-anthranthrene varied from 40 to 85 wt % as given in Tables 6A and 6B and the concentrations of the binder varied appropriately as also given in said Tables. The layer thicknesses are also given in Tables 6A and 6B.

The characteristics of the thus obtained photosensitive recording materials were determined as described above and are summarized together with those for EXAMPLE 1 in Tables 6A and 6B. The sensitivity to monochromatic 540 nm light exposure is expressed as the % discharge at an exposure ( $I_{540t}$ ) of 36.6 mJ/m<sup>2</sup> and the steepness of the discharge-exposure dependence is expressed as the % discharge observed between exposures ( $I_{540t}$ ) of 3.66 mJ/m<sup>2</sup> and 11.6 mJ/m<sup>2</sup> (see Table 6A) or between exposures ( $I_{540t}$ ) of 11.6 mJ/m<sup>2</sup> and 36.6 mJ/m<sup>2</sup> (see Table 6B) depending upon the sensitivity of the photosensitive recording material.

TABLE 6A-continued

| Comparative Example No. | Bis-             |                     | P1 conc. [wt %] | P2 conc. [wt %] | layer thickness [μm] | CL [V] | % discharge for $I_{540t} = 36.6 \text{ mJ/m}^2$ | % discharge between $I_{540t}$ 's of 3.66 and 11.6 $\text{mJ/m}^2$ |
|-------------------------|------------------|---------------------|-----------------|-----------------|----------------------|--------|--------------------------------------------------|--------------------------------------------------------------------|
|                         | DBA conc. [wt %] | fectol conc. [wt %] |                 |                 |                      |        |                                                  |                                                                    |
| 48                      | 60               | 5                   | 31.5            | 3.5             | 16                   | -654   | 97.9                                             | 85.0                                                               |
| 49                      | 70               | 3                   | 22.5            | 2.5             | 15                   | -530   | 98.1                                             | 73.6                                                               |
| 20                      | 85               | 5                   | 9.0             | 1.0             | 16                   | -176   | 96.0                                             | 29.5                                                               |

TABLE 6B

| Example No. | Bis-             |                     | P1 conc. [wt %] | P2 conc. [wt %] | layer thickness [μm] | CL [V] | % discharge for $I_{540t} = 36.6 \text{ mJ/m}^2$ | % discharge between $I_{540t}$ 's of 11.6 and 36.6 $\text{mJ/m}^2$ |
|-------------|------------------|---------------------|-----------------|-----------------|----------------------|--------|--------------------------------------------------|--------------------------------------------------------------------|
|             | DBA conc. [wt %] | fectol conc. [wt %] |                 |                 |                      |        |                                                  |                                                                    |
| 1           | 30               | 5                   | 58.5            | 6.5             | 12                   | -730   | 90.0                                             | 81.1                                                               |

## EXAMPLES 50 AND 51

The photosensitive recording materials of EXAMPLES 50 to 51 were produced as described for EXAMPLE 34 except that the concentrations of 4,10-dibromoanthanthrone were reduced to 10 and 8 wt % respectively and the concentrations of the binders were varied appropriately as given in Tables 7A and 7B. The layer thicknesses are given also in said Tables.

The characteristics of the thus obtained photosensitive recording materials were determined as described above and are summarized together with these for EXAMPLE 34 in Tables 7A and 7B. The sensitivity to monochromatic 540 nm light exposure is expressed as the % discharge at an exposure ( $I_{540t}$ ) of 116  $\text{mJ/m}^2$  and the steepness of the discharge-exposure dependence is expressed as the % discharge observed either between exposures ( $I_{540t}$ ) of 36.6  $\text{mJ/m}^2$  and 116  $\text{mJ/m}^2$  (see Table 7A) or between exposures ( $I_{540t}$ ) of 11.6  $\text{mJ/m}^2$  and 36.6  $\text{mJ/m}^2$  (see Table 7B) depending upon the sensitivity of the photosensitive recording material.

25 The photosensitive recording material of EXAMPLE 53 was produced as described for EXAMPLE 7 except that N,N'-bis(2,5-dimethyl-phenyl) perylimide was used as the sensitizing pigment instead of 4,10-dibromoanthanthrone C.I. Pigment Red 168 and CI 59 300. The layer thickness was 15  $\mu\text{m}$ . This photosensitive recording material exhibited 4.4% discharge upon  $I_{540t}$  exposure of 36.6  $\text{mJ/m}^2$  and 87.3% discharge between  $I_{540t}$  exposures of 36.6  $\text{mJ/m}^2$  and 116  $\text{mJ/m}^2$ .

## EXAMPLE 53

30 The photosensitive recording material of EXAMPLE 54 was produced as described for EXAMPLE 17 except that N,N'-bis(4-cyclohexyl-phenyl) perylimide was used as the sensitizing pigment instead of 4,10-dibromoanthanthrone C.I. Pigment Red 168 and CI 59 300. The layer thickness was 15  $\mu\text{m}$ . This photosensitive

35 The photosensitive recording material of EXAMPLE 54 was produced as described for EXAMPLE 17 except that N,N'-bis(4-cyclohexyl-phenyl) perylimide was used as the sensitizing pigment instead of 4,10-dibromoanthanthrone C.I. Pigment Red 168 and CI 59 300. The layer thickness was 15  $\mu\text{m}$ . This photosensitive

TABLE 7A

| Example No. | Bis-             |                     | P1 conc. [wt %] | P2 conc. [wt %] | layer thickness [μm] | CL [V] | % discharge for $I_{540t} = 116 \text{ mJ/m}^2$ | % discharge between $I_{540t}$ 's of 36.6 and 116 $\text{mJ/m}^2$ |
|-------------|------------------|---------------------|-----------------|-----------------|----------------------|--------|-------------------------------------------------|-------------------------------------------------------------------|
|             | DBA conc. [wt %] | fectol conc. [wt %] |                 |                 |                      |        |                                                 |                                                                   |
| 34          | 25               | 10                  | 58.5            | 6.5             | 14                   | -835   | 96.4                                            | —                                                                 |
| 50          | 10               | 10                  | 72.0            | 8.0             | 17                   | -863   | 70.5                                            | 56.2                                                              |
| 51          | 8                | 10                  | 73.8            | 8.2             | 12                   | -725   | 83.3                                            | 56.8                                                              |

TABLE 7B

| Example No. | Bis-             |                     | P1 conc. [wt %] | P2 conc. [wt %] | layer thickness [μm] | CL [V] | % discharge for $I_{540t} = 116 \text{ mJ/m}^2$ | % discharge between $I_{540t}$ 's of 11.6 and 36.6 $\text{mJ/m}^2$ |
|-------------|------------------|---------------------|-----------------|-----------------|----------------------|--------|-------------------------------------------------|--------------------------------------------------------------------|
|             | DBA conc. [wt %] | fectol conc. [wt %] |                 |                 |                      |        |                                                 |                                                                    |
| 34          | 25               | 10                  | 58.5            | 6.5             | 14                   | -835   | 96.4                                            | 85.3                                                               |

## EXAMPLE 52

The photosensitive recording material of EXAMPLE 52 was produced as described for EXAMPLE 7 except that N,N'-bis(4-methyl-phenyl) perylimide was used as the sensitizing pigment instead of 4,10-dibromoanthanthrone C.I. Pigment Red 168 and CI 59 300. The layer thickness was 14  $\mu\text{m}$ . This photosensitive recording material exhibited 5.7% discharge upon  $I_{540t}$  expo-

60 recording material exhibited 3.8% discharge upon  $I_{575t}$  exposure of 53.8  $\text{mJ/m}^2$  and 54.7% discharge between  $I_{575t}$  exposures of 53.8  $\text{mJ/m}^2$  and 170  $\text{mJ/m}^2$ .

## EXAMPLE 55

65 The photosensitive recording material of EXAMPLE 55 was produced as described for EXAMPLE 7 except that N,N'-bis(3-methyl-phenyl) perylimide was used as the sensitizing pigment instead of 4,10-dibromoanthanthrone C.I. Pigment Red 168 and CI 59 300. The

layer thickness was 13  $\mu\text{m}$ . This photosensitive recording material exhibited 6.9% discharge upon  $I_{575t}$  exposure of 53.8  $\text{mJ}/\text{m}^2$  and 55.6% discharge between  $I_{575t}$  exposures of 53.8  $\text{mJ}/\text{m}^2$  and 170  $\text{mJ}/\text{m}^2$ .

#### EXAMPLE 56

The photosensitive recording material of EXAMPLE 56 was produced as described for EXAMPLE 17 except that N,N'-bis(2,3,5-trimethyl-phenyl) perylimide was used as the sensitizing pigment instead of 4,10-dibromo anthanthrone C.I. Pigment Red 168 and CI 300. The layer thickness was 15  $\mu\text{m}$ . This photosensitive recording material exhibited 1.2% discharge upon  $I_{540t}$  exposure of 36.6  $\text{mJ}/\text{m}^2$  and 71.8% discharge between  $I_{540t}$  exposures of 36.6  $\text{mJ}/\text{m}^2$  and 116  $\text{mJ}/\text{m}^2$ .

#### EXAMPLE 57

The photosensitive recording material of EXAMPLE 57 was produced by first doctor blade coating a 100  $\mu\text{m}$  thick polyester film precoated with a vacuum-deposited conductive layer of aluminium with a 1% solution of  $\gamma$ -aminopropyltriethoxy silane in aqueous methanol. After evaporating the solvent and curing the resulting adhesion/blocking layer at 100° C. for 30 minutes, the adhesion/blocking layer was overcoated with a dispersion of charge generating pigment containing charge transport material to a thickness of 16  $\mu\text{m}$ .

Said dispersion was prepared by mixing 2 g of 4,10-dibromo-anthanthrone, 0.78 g of aromatic polycarbonate MAKROLON CD 2000 (registered trade mark) and 20.38 g of dichloromethane for 15 minutes in a pearl mill. 0.8 g of  $\alpha,\alpha'$ -bis (6-ethoxy-1,2-dihydro-2,2,4-trimethyl-quinolin-1-yl)-p-xylene, 4.42 g of MAKROLON CD 2000 (registered trade mark) and 11.6 g of dichloromethane were then added and the resulting mixture mixed for a further 5 minutes to produce the composition and viscosity for casting.

The photosensitive layer was then dried for 16 hours at 50° C.

The characteristics of the thus obtained photosensitive recording material were determined as described above. The sensitivity to monochromatic 540 nm light exposure is expressed as the % discharge at an exposure ( $I_{540t}$ ) of 38  $\text{mJ}/\text{m}^2$  and the steepness of the discharge-exposure dependence is expressed as the % discharge observed between exposures ( $I_{540t}$ ) of 12  $\text{mJ}/\text{m}^2$  and 38

#### EXAMPLES 58 TO 61 AND COMPARATIVE EXAMPLE 21

In the production of EXAMPLES 58 to 61 and COMPARATIVE EXAMPLE 21 a 100  $\mu\text{m}$  thick polyester film precoated with a vacuum-deposited conductive layer of aluminium was doctor-blade coated with a dispersion of charge generating pigment containing charge transport material to thicknesses given in Table 8.

Said dispersion was prepared by mixing for 15 minutes in a pearl mill 2.5 g of 4,10-dibromoanthanthrone, 5.85 g of an aromatic polycarbonate MAKROLON CD 2000 (registered trade mark) (P1), 0.65 g of a polyester adhesion promoting additive DYNAPOL L206 (registered trade mark) (P2) and 35.45 g of dichloromethane and subsequently adding 1.0 g of a mixture of 1,2-bis(1,2-dihydro-2,2,4-trimethyl-quinolin-1-yl)ethane (Bisflectol) and tris(p-tolyl)amine (TTA) in the proportions given in Table 8 and mixing for a further 5 minutes.

The resulting layer was dried for 16 hours at 50° C.

The half-wave oxidation potentials versus s.c.e. of Bisflectol and TTA determined as described above were 0.694 V and 0.772 V respectively, a difference of 0.078 V.

The characteristics of the thus obtained photosensitive recording materials were determined as described above. The sensitivity to monochromatic 540 nm light exposure is expressed as the % discharge at an exposure ( $I_{540t}$ ) of 38  $\text{mJ}/\text{m}^2$  and the steepness of the discharge-exposure dependence is expressed as the % discharge observed between exposures ( $I_{540t}$ ) of 12  $\text{mJ}/\text{m}^2$  and 38  $\text{mJ}/\text{m}^2$ , a factor of 3.16 difference in exposure. The results are summarized in Table 8.

Sensitometric measurements were carried out using the refined sensitometric measurement techniques described above. The resulting sensitometric curves for the photosensitive layers of EXAMPLES 58, 59, 60 and 61 and COMPARATIVE EXAMPLE 21 are shown in FIGS. 6, 7, 8, 9 and 10 respectively. The exposures required for 10% and 90% discharges differ by factors of 2.8, 2.7, 2.7, 2.5 and >3.8 for the photosensitive layers of EXAMPLE 58, EXAMPLE 59, EXAMPLE 60, EXAMPLE 61, and COMPARATIVE EXAMPLE 21 respectively.

TABLE 8

| Example No.             | DBA conc. [wt %] | Bis-flectol conc. [wt %] | TTA conc. [wt %] | P1 conc. [wt %] | P2 conc. [wt %] | layer thickness [ $\mu\text{m}$ ] | CL [V] | % discharge for $I_{540t} = 38 \text{ mJ}/\text{m}^2$ | % discharge between $I_{540t}$ 's of 12 and 38 $\text{mJ}/\text{m}^2$ |
|-------------------------|------------------|--------------------------|------------------|-----------------|-----------------|-----------------------------------|--------|-------------------------------------------------------|-----------------------------------------------------------------------|
| 58                      | 25               | 10                       | 0                | 58.5            | 6.5             | 14                                | -671   | 94.3                                                  | 80.8                                                                  |
| 59                      | 25               | 8                        | 2                | 58.5            | 6.5             | 14                                | -662   | 95.5                                                  | 79.3                                                                  |
| 60                      | 25               | 5                        | 5                | 58.5            | 6.5             | 17                                | -707   | 93.5                                                  | 76.9                                                                  |
| 61                      | 25               | 2                        | 8                | 58.5            | 6.5             | 13                                | -689   | 94.2                                                  | 82.4                                                                  |
| COMPARATIVE EXAMPLE No. |                  |                          |                  |                 |                 |                                   |        |                                                       |                                                                       |
| 21                      | 25               | 0                        | 10               | 58.5            | 6.5             | 14                                | -711   | 67.5                                                  | 55.7                                                                  |

$\text{mJ}/\text{m}^2$ , a factor of 3.16 difference in exposure:

% discharge for  $I_{540t} = 38 \text{ mJ}/\text{m}^2$ : 89.2

% discharge between  $I_{540t}$ 's of 12  $\text{mJ}/\text{m}^2$  and 38  $\text{mJ}/\text{m}^2$ :

72.4.

65

#### EXAMPLES 62 and 63 and COMPARATIVE EXAMPLE 22

The photosensitive recording materials of EXAMPLES 62 and 63 and COMPARATIVE EXAMPLE 22 were produced as described for EXAMPLES 58 to 61

and COMPARATIVE EXAMPLE 21 except that 2,5-bis(4-N,N-diethylaminophenyl)oxadiazole-1,3,4 (OXA) was substituted for tris(p-tolyl)amine. The compositions and layer thickness of the resulting photosensitive recording materials are given in TABLE 9.

The half-wave oxidation potentials versus s.c.e. of Bisflectol and OXA determined as described above were 0.694 V and 0.87 V respectively, a difference of 0.176 V.

The characteristics of the thus obtained photosensitive recording materials were determined as described above. The sensitivity to monochromatic 540 nm light exposure is expressed as the % discharge at an exposure ( $I_{540t}$ ) of 38 mJ/m<sup>2</sup> and the steepness of the discharge exposure dependence is expressed as the % discharge observed between exposures ( $I_{540t}$ ) of 12 mJ/m<sup>2</sup> and 38 mJ/m<sup>2</sup> a factor of 3.16 difference in exposure. The results are summarized together with those for EXAMPLE 58 in TABLE 10.

Sensitometric measurements were carried out using the refined sensitometric measurement techniques described above. The resulting sensitometric curve for the photosensitive layer of EXAMPLE 64 is shown in FIG.

15 14. The exposures required for 10% and 90% discharge differ by a factor of 4.3 compared with 2.8 for EXAMPLE 58 (FIG. 6).

TABLE 10

| Example No. | DBA conc. [wt %] | Bis-flectol conc. [wt %] | DEH conc. [wt %] | P1 conc. [wt %] | P2 conc. [wt %] | layer thickness [μm] | CL [V] | % discharge for $I_{540t} = 38$ mJ/m <sup>2</sup> | % discharge between $I_{540t}$ 's of 12 and 38 mJ/m <sup>2</sup> |
|-------------|------------------|--------------------------|------------------|-----------------|-----------------|----------------------|--------|---------------------------------------------------|------------------------------------------------------------------|
| 58          | 25               | 10                       | 0                | 58.5            | 6.5             | 14                   | -671   | 94.3                                              | 80.8                                                             |
| 64          | 25               | 5                        | 5                | 58.5            | 6.5             | 13                   | -691   | 91.9                                              | 62.1                                                             |

sults are summarized together with those for EXAMPLE 58 in TABLE 9 below.

Sensitometric measurements were carried out using the refined sensitometric measurement techniques described above. The resulting sensitometric curves for the photosensitive layers of EXAMPLES 62 and 63 and COMPARATIVE EXAMPLE 22 are shown in FIGS. 11, 12 and 13. The exposures required for 10% and 90% discharge differ by factors of 2.6 and 2.5 for EXAMPLE 62 and EXAMPLE 63 respectively compared with 2.8 for EXAMPLE 58 (FIG. 6), and 4.7 for COMPARATIVE EXAMPLE 22.

30 The photosensitive recording material of EXAMPLE 65 was produced as described for EXAMPLE 60 except that 1,2-bis(1,2-dihydro-2,4,6,7-pentamethyl-quinolin-1-yl)ethane (DH) was substituted for tris(p-tolyl)amine and the layer thickness was 10 μm instead of 17 μm.

35 The half-wave oxidation potentials versus s.c.e. of Bisflectol and DH determined as described above were 0.694 V and 0.595 V respectively, corresponding to a difference of 0.099 V.

TABLE 9

| Example No.             | DBA conc. [wt %] | Bis-flectol conc. [wt %] | OXA conc. [wt %] | P1 conc. [wt %] | P2 conc. [wt %] | layer thickness [μm] | CL [V] | % discharge for $I_{540t} = 38$ mJ/m <sup>2</sup> | % discharge between $I_{540t}$ 's of 12 and 38 mJ/m <sup>2</sup> |
|-------------------------|------------------|--------------------------|------------------|-----------------|-----------------|----------------------|--------|---------------------------------------------------|------------------------------------------------------------------|
| 58                      | 25               | 10                       | 0                | 58.5            | 6.5             | 14                   | -671   | 94.3                                              | 90.8                                                             |
| 62                      | 25               | 5                        | 5                | 58.5            | 6.5             | 16                   | -586   | 95.9                                              | 58.5                                                             |
| 63                      | 25               | 2                        | 8                | 58.5            | 6.5             | 14                   | -657   | 96.5                                              | 57.7                                                             |
| COMPARATIVE EXAMPLE No. |                  |                          |                  |                 |                 |                      |        |                                                   |                                                                  |
| 22                      | 25               | 0                        | 10               | 58.5            | 6.5             | 10                   | -627   | 97.0                                              | 68.6                                                             |

EXAMPLE 64

The photosensitive recording material of EXAMPLE 64 was produced as described for EXAMPLES 58 to 61 and COMPARATIVE EXAMPLE 21 except that 4-N,N-diethylaminobenzaldehyde-1',1'-diphenylhydrazone (DEH) was substituted for tris(p-tolyl)amine. The compositions and layer thickness of the resulting photosensitive recording materials are given in TABLE 10.

The half-wave oxidation potentials versus s.c.e. of Bisflectol and DEH determined as described above were 0.694 V and 0.538 V respectively, a difference of 0.156 V.

55 The characteristics of the thus obtained photosensitive recording materials were determined as described above. The sensitivity to monochromatic 540 nm light exposure is expressed as the % discharge at an exposure ( $I_{540t}$ ) of 38 mJ/m<sup>2</sup> and the steepness of the discharge-exposure dependence is expressed as the % discharge observed between exposures ( $I_{540t}$ ) of 12 mJ/m<sup>2</sup> and 38 mJ/m<sup>2</sup> a factor of 3.16 difference in exposure. The results are summarized together with those example 58 in TABLE 11 below.

60 Sensitometric measurements were carried out using the refined sensitometric measurement techniques described above. The resulting sensitometric curve for the photosensitive layer of EXAMPLES 65 shown in FIG. 15. The exposures required for 10% and 90% discharge differ by a factor of 4.0.

TABLE 11

| Example No. | DBA conc. [wt %] | Bis-flectol conc. [wt %] | DH conc. [wt %] | P1 conc. [wt %] | P2 conc. [wt %] | layer thickness [μm] | CL [V] | % discharge for $I_{540t} = 38 \text{ mJ/m}^2$ | % discharge between $I_{540t}$ 's of 12 and $38 \text{ mJ/m}^2$ |
|-------------|------------------|--------------------------|-----------------|-----------------|-----------------|----------------------|--------|------------------------------------------------|-----------------------------------------------------------------|
| 58          | 25               | 10                       | 0               | 58.5            | 6.5             | 14                   | -671   | 94.3                                           | 80.8                                                            |
| 65          | 25               | 5                        | 5               | 58.5            | 6.5             | 10                   | -488   | 92.8                                           | 80.5                                                            |

## COMPARATIVE EXAMPLE 23

The photosensitive material of COMPARATIVE EXAMPLE 23 was produced as described for EXAMPLE 7 except that the charge transport material N-(4-N,N-dibenzylphenyl)-carbazole (DPPC) was used instead of Bisflectol and the layer thickness was 14  $\mu\text{m}$  instead of 10  $\mu\text{m}$ .

The characteristics of the thus obtained photosensi-

10 sults are summarized together with those for EXAMPLE 58 and COMPARATIVE EXAMPLE 23 in TABLE 12 below.

Sensitometric measurements were carried out using the refined sensitometric measurement techniques described above. The resulting sensitometric curve for the photosensitive layers of EXAMPLE 66 shown in FIG. 16. The exposures required for 10% and 90% discharge differ by a factor of 2.2.

TABLE 12

| Example No.             | DBA conc. [wt %] | Bis-flectol conc. [wt %] | DPPC conc. [wt %] | P1 conc. [wt %] | P2 conc. [wt %] | layer thickness [μm] | CL [V] | % discharge for $I_{540t} = 38 \text{ mJ/m}^2$ | % discharge between $I_{540t}$ 's of 12 and $38 \text{ mJ/m}^2$ |
|-------------------------|------------------|--------------------------|-------------------|-----------------|-----------------|----------------------|--------|------------------------------------------------|-----------------------------------------------------------------|
| 58                      | 25               | 10                       | 0                 | 58.5            | 6.5             | 14                   | -671   | 94.3                                           | 80.8                                                            |
| 66                      | 25               | 5                        | 5                 | 58.5            | 6.5             | 14                   | -554   | 94.2                                           | 81.4                                                            |
| COMPARATIVE EXAMPLE No. |                  |                          |                   |                 |                 |                      |        |                                                |                                                                 |
| 23                      | 25               | 0                        | 10                | 58.5            | 6.5             | 14                   | -892   | 82.1                                           | 72.3                                                            |

tive recording materials were determined as described above. The sensitivity to monochromatic 540 nm light exposure is expressed as the % discharge at an exposure ( $I_{540t}$ ) of 36.6  $\text{mJ/m}^2$  and the steepness of the discharge-exposure dependence is expressed as the % discharge observed between exposures ( $I_{540t}$ ) of 11.6  $\text{mJ/m}^2$  and 36.6  $\text{mJ/m}^2$  a factor of 3.16 difference in exposure. The residual potential for an exposure ( $I_{540t}$ ) of 116  $\text{mJ/m}^2$  -104 V was greater than 10% of the charging 40 level: -892 V indicating that the exposures required for 10% and 90% discharge differ by a factor > 10.

## EXAMPLE 66

The photosensitive recording material of EXAMPLE 66 was produced as described for EXAMPLE 60 except that DPPC was substituted for TTA and the layer thickness was 14  $\mu\text{m}$  instead of 17  $\mu\text{m}$ .

The half-wave oxidation potentials versus s.c.e. of Bisflectol and DPPC determined as described above 50 were 0.694 and 0.915 V respectively, corresponding to a difference of 0.221 V.

The characteristics of the thus obtained photosensitive recording materials were determined as described above. The sensitivity to monochromatic 540 nm light exposure is expressed as the % discharge at an exposure ( $I_{540t}$ ) of 38  $\text{mJ/m}^2$  and the steepness of the discharge-exposure dependence is expressed as the % discharge observed between exposures ( $I_{540t}$ ) of 12  $\text{mJ/m}^2$  and 38  $\text{mJ/m}^2$  a factor of 3.16 difference in exposure. The re- 60

35 sults are summarized together with those for EXAMPLE 57 and comparative EXAMPLE 22 in TABLE 13. The photosensitive recording material of EXAMPLE 67 was produced as described for EXAMPLE 60 except that  $\alpha,\alpha'$ -bis(6-ethoxy-1,2-dihydro-2,4-trimethyl quinolin-1-yl) p-xylene (EQX) and OXA have been substituted for Bisflectol and TTA and that the layer thickness layer of the photosensitive recording material was 16  $\mu\text{m}$  instead of 17  $\mu\text{m}$ .

The half-wave oxidation potentials versus s.c.e. of EQX and OXA determined as described above were 0.540 V and 0.870 V respectively, a difference of 0.330 V.

The characteristics of the thus obtained photosensitive recording materials were determined as described above. The sensitivity to monochromatic 540 nm light exposure is expressed as the % discharge at an exposure ( $I_{540t}$ ) of 38  $\text{mJ/m}^2$  and the steepness of the discharge-exposure dependence is expressed as the % discharge observed between exposures ( $I_{540t}$ ) of 12  $\text{mJ/m}^2$  and 38  $\text{mJ/m}^2$  a factor of 3.16 difference in exposure. The results are summarize together with those for EXAMPLE 57 and comparative EXAMPLE 22 in TABLE 13.

Sensitometric measurements were carried out using the refined sensitometric measurement techniques described above. The resulting sensitometric curve for the photosensitive layer of EXAMPLE 67 is shown in FIG. 17. The exposures required for 10% and 90% discharge differ by a factor of 2.7.

TABLE 13

| Example No. | DBA conc. [wt %] | EQX conc. [wt %] | OXA conc. [wt %] | P1 conc. [wt %] | P2 conc. [wt %] | layer thickness [μm] | CL [V] | % discharge for $I_{540t} = 38 \text{ mJ/m}^2$ | % discharge between $I_{540t}$ 's of 12 and $38 \text{ mJ/m}^2$ |
|-------------|------------------|------------------|------------------|-----------------|-----------------|----------------------|--------|------------------------------------------------|-----------------------------------------------------------------|
| 57          | 25               | 10               | 0                | 58.5            | 6.5             | 16                   | -845   | 89.2                                           | 72.4                                                            |

TABLE 13-continued

|                                     | DBA<br>conc.<br>[wt %] | EQX<br>conc.<br>[wt %] | OXA<br>conc.<br>[wt %] | P1<br>conc.<br>[wt %] | P2<br>conc.<br>[wt %] | layer<br>thickness<br>[μm] | CL<br>[V] | % discharge<br>for $I_{540t} =$<br>38 mJ/m <sup>2</sup> | % discharge<br>between $I_{540t}$ 's<br>of 12 and<br>38 mJ/m <sup>2</sup> |
|-------------------------------------|------------------------|------------------------|------------------------|-----------------------|-----------------------|----------------------------|-----------|---------------------------------------------------------|---------------------------------------------------------------------------|
| 67<br>COMPARATIVE<br>EXAMPLE<br>No. | 25                     | 5                      | 5                      | 58.5                  | 6.5                   | 16                         | -267      | 82.0                                                    | 34.1                                                                      |
| 22                                  | 25                     | 0                      | 10                     | 58.5                  | 6.5                   | 10                         | -627      | 97.0                                                    | 68.6                                                                      |

## EXAMPLE 68

The photosensitive recording material of EXAMPLE 68 was produced as described for EXAMPLE 67 except that DEH was substituted for OXA and the layer thickness was 13 μm instead of 16 μm.

The half-wave oxidation potentials versus s.c.e. of EQX and DEH determined as described above were 0.540 V and 0.538 V respectively a difference of 0.002 V.

The characteristics of the thus obtained photosensitive recording materials were determined as described above. The sensitivity to monochromatic 540 nm light exposure is expressed as the % discharge at an exposure

above. The sensitivity to monochromatic 540 nm light exposure is expressed as the % discharge at an exposure ( $I_{540t}$ ) of 38 mJ/m<sup>2</sup> and the steepness of the discharge-exposure dependence is expressed as the % discharge observed between exposures ( $I_{540t}$ ) of 12 mJ/m<sup>2</sup> and 38 mJ/m<sup>2</sup> a factor of 3.16 difference in exposure. The results are summarized together with those EXAMPLE 57 in TABLE 15 below.

Sensitometric measurements were carried out using the refined sensitometric measurement techniques described above. The resulting sensitometric curve for the photosensitive layer of EXAMPLE 69 shown in FIG. 19. The exposures required for 10% and 90% discharge differ by a factor of 4.4

TABLE 15

| Example<br>No. | DBA<br>conc.<br>[wt %] | EQX<br>conc.<br>[wt %] | DH<br>conc.<br>[wt %] | P1<br>conc.<br>[wt %] | P2<br>conc.<br>[wt %] | layer<br>thickness<br>[μm] | CL<br>[V] | % discharge<br>for $I_{540t} =$<br>38 mJ/m <sup>2</sup> | % discharge<br>between $I_{540t}$ 's<br>of 12 and<br>38 mJ/m <sup>2</sup> |
|----------------|------------------------|------------------------|-----------------------|-----------------------|-----------------------|----------------------------|-----------|---------------------------------------------------------|---------------------------------------------------------------------------|
| 57             | 25                     | 10                     | 0                     | 58.5                  | 6.5                   | 16                         | -845      | 89.2                                                    | 72.4                                                                      |
| 69             | 25                     | 5                      | 5                     | 58.5                  | 6.5                   | 10                         | -455      | 90.5                                                    | 76.3                                                                      |

( $I_{540t}$ ) of 38 mJ/m<sup>2</sup> and the steepness of the discharge-exposure dependence is expressed as the % discharge observed between exposures ( $I_{540t}$ ) of 12 mJ/m<sup>2</sup> and 38 mJ/m<sup>2</sup> a factor of 3.16 difference in exposure. The results are summarized together with those EXAMPLE 57 in TABLE 9 below.

Sensitometric measurements were carried out using the refined sensitometric measurement techniques described above. The resulting sensitometric curve for the photosensitive layer of EXAMPLE 68 shown in FIG. 18. The exposures required for 10% and 90% discharge differ by a factor of 2.16.

## EXAMPLE 70 AND COMPARATIVE EXAMPLE 24

The photosensitive recording materials of EXAMPLE 70 and COMPARATIVE EXAMPLE 24 were produced as described for EXAMPLE 60 and COMPARATIVE EXAMPLE 21 respectively except that 1,3,5-tris[4-N,N-bis(4-ethylphenyl)aminophenyl]-benzene (TEPAB) was substituted for Bisflectol in the case of EXAMPLE 70 and for OXA in the case of COMPARATIVE EXAMPLE 24 and the layer thickness were 10 μm instead of 17 μm and 16 μm instead of 14

TABLE 14

| Example<br>No. | DBA<br>conc.<br>[wt %] | EQX<br>conc.<br>[wt %] | DEH<br>conc.<br>[wt %] | P1<br>conc.<br>[wt %] | P2<br>conc.<br>[wt %] | layer<br>thickness<br>[μm] | CL<br>[V] | % discharge<br>for $I_{540t} =$<br>38 mJ/m <sup>2</sup> | % discharge<br>between $I_{540t}$ 's<br>of 12 and<br>38 mJ/m <sup>2</sup> |
|----------------|------------------------|------------------------|------------------------|-----------------------|-----------------------|----------------------------|-----------|---------------------------------------------------------|---------------------------------------------------------------------------|
| 57             | 25                     | 10                     | 0                      | 58.5                  | 6.5                   | 16                         | -845      | 89.2                                                    | 72.4                                                                      |
| 68             | 25                     | 5                      | 5                      | 58.5                  | 6.5                   | 13                         | -665      | 94.4                                                    | 78.8                                                                      |

## EXAMPLE 69

The photosensitive recording material of EXAMPLE 69 was produced as described for EXAMPLE 67 except that 1,2-bis(1,2-dihydro-2,2,4,6,7-pentamethyl-quinolin-1-yl)ethane (DH) had been substituted for OXA and the layer thickness was 10 μm instead of 16 μm.

The half-wave oxidation potentials versus s.c.e. of EQX and 1,2-bis(1,2-dihydro-2,2,4,6,7-pentamethyl-quinolin-1-yl)-ethane determined as described above were 0.540 V and 0.595 V respectively, corresponding with a difference of 0.055 V.

The characteristics of the thus obtained photosensitive recording materials were determined as described

55 μm respectively.

The half-wave oxidation potentials versus s.c.e. of TEPAB and OXA determined as described above were 0.885 V and 0.870 V respectively, a difference of 0.015 V.

The characteristics of the thus obtained photosensitive recording materials were determined as described above. The sensitivity to monochromatic 540 nm light exposure is expressed as the % discharge at an exposure ( $I_{540t}$ ) of 38 mJ/m<sup>2</sup> and the steepness of the discharge-exposure dependence is expressed as the % discharge observed between exposures ( $I_{540t}$ ) of 12 mJ/m<sup>2</sup> and 38 mJ/m<sup>2</sup> a factor of 3.16 difference in exposure. The re-

sults are summarized together with those for COMPARATIVE EXAMPLE 27 in TABLE 16 below.

Sensitometric measurements were carried out using the refined sensitometric measurement techniques described above. The resulting sensitometric curve for the photosensitive layer of EXAMPLE 70 and COMPARATIVE EXAMPLE 24 are shown in FIGS. 20 and 21. The exposures required for 10% and 90% discharge differ by factors of 3.3 and >>1.9 for the photosensitive layers of EXAMPLE 70 and COMPARATIVE EXAMPLE 24 respectively.

layer has a thickness in the range of 4 to 40  $\mu\text{m}$  and comprises 8 to 80% by weight of said n-type pigment substance and 0.01 to 40% by weight of said p-type charge transport substance that is molecularly distributed in said electrically insulating organic polymeric binder material that has a volume resistivity of at least  $10^{14}$  Ohm-m, and wherein said recording layer in electrostatically charged state requires for 10% and 90% discharge respectively exposures to conductivity increasing electromagnetic radiation that differ by a factor 4.5 or less, and wherein at least one p-type charge

TABLE 16

| Example No.             | DBA conc. [wt %] | TEPAB conc. [wt %] | OXA conc. [wt %] | P1 conc. [wt %] | P2 conc. [wt %] | layer thickness [ $\mu\text{m}$ ] | CL [V] | % discharge for $I_{540t} = 38 \text{ mJ/m}^2$ | % discharge between $I_{540t}$ 's of 12 and 38 $\text{mJ/m}^2$ |
|-------------------------|------------------|--------------------|------------------|-----------------|-----------------|-----------------------------------|--------|------------------------------------------------|----------------------------------------------------------------|
| 70                      | 25               | 5                  | 5                | 58.5            | 6.5             | 10                                | -532   | 96.4                                           | 74.4                                                           |
| COMPARATIVE EXAMPLE No. |                  |                    |                  |                 |                 |                                   |        |                                                |                                                                |
| 22                      | 25               | 0                  | 10               | 58.5            | 6.5             | 10                                | -627   | 97.0                                           | 68.6                                                           |
| 24                      | 25               | 10                 | 0                | 58.5            | 6.5             | 16                                | -749   | 18.6                                           | 13.4                                                           |

## EXAMPLES 71 TO 73

The photosensitive recording materials of EXAMPLES 71 to 73 were produced as described for EXAMPLE 58 except that in all cases the Bisflectol concentration has been increased and in two cases the DBA concentration was been varied with corresponding adjustments to the P1 and P2 concentrations. The DBA, Bisflectol, P1 and P2 concentrations are given in Tables 17 together with the photosensitive recording material layer thicknesses.

The characteristics of the thus obtained photosensitive recording materials were determined as described above. The sensitivity to monochromatic 540 nm light exposure is expressed as the % discharge at an exposure ( $I_{540t}$ ) of 38  $\text{mJ/m}^2$  and the steepness of the discharge-exposure dependence is expressed as the % discharge observed between exposures ( $I_{540t}$ ) of 12  $\text{mJ/m}^2$  and 38  $\text{mJ/m}^2$  a factor of 3.16 difference in exposure. The results are summarized together with those for EXAMPLES 4, 9, 10, 15 and 19 to 21 in TABLE 17 below.

TABLE 17

| Example No. | DBA conc. [wt %] | Bisflectol conc. [wt %] | P1 conc. [wt %] | P2 conc. [wt %] | layer thickness [ $\mu\text{m}$ ] | CL [V] | % discharge for $I_{540t} = 38 \text{ mJ/m}^2$ | % discharge between $I_{540t}$ 's of 12 and 38 $\text{mJ/m}^2$ |
|-------------|------------------|-------------------------|-----------------|-----------------|-----------------------------------|--------|------------------------------------------------|----------------------------------------------------------------|
| 4           | 30               | 30                      | 36              | 4.0             | 10                                | -574   | 93.0                                           | 56.4                                                           |
| 71          | 25               | 21                      | 48.6            | 5.4             | 13                                | -692   | 85.0                                           | 66.9                                                           |
| 72          | 25               | 23                      | 46.8            | 5.2             | 12                                | -656   | 90.9                                           | 69.2                                                           |
| 9           | 25               | 25                      | 45              | 5.0             | 11                                | -640   | 95.8                                           | 70.9                                                           |
| 10          | 25               | 30                      | 40.5            | 5.6             | 8                                 | -524   | 96.6                                           | 60.9                                                           |
| 73          | 20               | 21                      | 53.1            | 5.9             | 12                                | -685   | 80.0                                           | 61.5                                                           |
| 15          | 20               | 30                      | 45              | 5.0             | 11                                | -636   | 90.3                                           | 63.1                                                           |
| 20          | 16               | 24                      | 54              | 6.0             | 10                                | -617   | 82.2                                           | 54.5                                                           |
| 19          | 15               | 20                      | 58.5            | 6.5             | 11                                | -697   | 66.1                                           | 44.6                                                           |
| 21          | 15               | 30                      | 49.5            | 5.5             | 8                                 | -606   | 81.2                                           | 48.2                                                           |

We claim:

1. An electrophotographic recording material comprising on an electrically conductive support a negatively chargeable photoconductive recording layer which contains in an electrically insulating organic polymeric binder material at least one photoconductive n-type pigment substance and one or more p-type photoconductive charge transport substances, wherein said

transport substance corresponds to a following general formula (I):



wherein:

R is a member selected from the group consisting of hydrogen, an aliphatic group, and a cycloaliphatic group including these groups substituted by non-ionic substituents, each of R<sup>1</sup> and R<sup>2</sup> (same or different) is a member selected from the group consisting of a C<sub>1</sub>-C<sub>6</sub> alkyl group, and an aryl group, and

Z are the atoms selected from the group consisting of those necessary to close an adjacent aromatic nu-

cleus, and an aromatic ring system including such nucleus or ring system substituted with one or more substituents of non-ionic character; and formula (II):



wherein:

X is a member selected from the group consisting of a bivalent aliphatic, a cycloaliphatic group, an alkylene chain interrupted by a bivalent aromatic group, and a bivalent aliphatic group wherein at least two carbon atoms are linked through a heteroatom selected from the group consisting of oxygen, sulphur and nitrogen wherein nitrogen is substituted with a monovalent hydrocarbon group, and R<sup>1</sup>, R<sup>2</sup> and Z have the same significance as described for general formula (I).

2. An electrophotographic recording material according to claim 1, wherein in said recording layer a mixture is present of different p-type charge transport substances including at least one substance according to a said general formula (I) to (V), and wherein the mixed p-type transport substances have half-wave oxidation potentials that do not differ by more than 0.4 V.

3. An electrophotographic recording material according to claim 1 or 2, wherein the support of said photoconductive recording layer is pre-coated with an adhesive and/or a blocking layer.

4. An electrophotographic recording material according to claim 1, wherein the photoconductive recording layer is overcoated with an outermost protective layer.

5. An electrophotographic recording material according to claim 1, wherein said recording material has an outermost binder layer containing at least one p-type transport substance being not admixed with said photoconductive n-type pigment(s).

6. An electrophotographic recording material according to claim 5, wherein said outermost layer has a thickness not larger than 7  $\mu\text{m}$ .

7. An electrophotographic recording material according to claim 1, wherein said recording layer has a thickness in the range of 5 to 35  $\mu\text{m}$  and contains 10 to 70% by weight of said n-type pigment substance and 1 to 30% by weight of said p-type charge transport substance(s).

8. An electrophotographic recording material according to claim 1, wherein said recording layer has a thickness in the range of 5 to 35  $\mu\text{m}$  and contains 50 to 80% by weight of said n-type pigment substance and 0.01 to 10% by weight of said p-type charge transport substance(s).

9. An electrophotographic recording material according to claim 1, wherein said recording layer has a thickness in the range of 5 to 35  $\mu\text{m}$  and contains 15 to 30% by weight of said n-type pigment substance and between 20 and 30% by weight of said p-type charge transport substance(s).

10. An electrophotographic recording material according to claim 2, wherein the admixed p-type charge transport substance(s) being different from the ones represented by a said general formula (I) and (II) is a member selected from the group consisting of:

i) triphenylamines,

- ii) tetra-N,N,N',N'-tetraphenylbenzidines,
- iii) hydrazones,
- iv) pyrazolines,
- v) oxadiazoles,
- vi) triarylmethanes.

11. An electrophotographic recording material according to claim 2, wherein the admixed p-type charge transport substance(s) being different from the ones represented by a said general formula (I) and II is a member selected from the group consisting of:

- i) poly(vinylcarbazoles),
- ii) poly(vinylpolycyclic aromatics),
- iii) pyrene-formaldehyde condensation polymers,
- iv) polyxylylenes,
- v) polymeric 1,2-dihydro-2,2,4-trimethylquinolines,
- vi) polymeric tetraphenylbenzidines and triphenylamines.

12. An electrophotographic recording material according to claim 1 wherein the n-type pigment(s) is a member selected from the group consisting of:

- a) perylimides,
- b) polynuclear quinones,
- c) quinacridones,
- d) naphthalene 1,4,5,8-tetracarboxylic acid derived pigments including the perinones,
- e) n-type indigo and thioindigo dyes,
- f) perylene 3,4,9,10-tetracarboxylic acid derived pigments including condensation products with o-diamines,
- g) n-type polyazo-pigments including bisazo-, trisazo- and tetrakisazo-pigments.

13. An electrophotographic recording material according to claim 1, wherein the polymeric binder is an organic resin material selected from the group consisting of a cellulose ester, acrylate and methacrylate resin, polyvinyl chloride, copolymers of vinyl chloride, copolyvinyl chloride/acetate and copolyvinylchloride/maleic anhydride, polyester resin, aromatic polycarbonate resin and polyester carbonate resin.

14. An electrophotographic recording material according to claim 1, wherein the polymeric binder is an aromatic polycarbonate having in its structure repeating units within the scope of the following general formula:



wherein:

X is a member selected from the group consisting of S,



each of R<sup>31</sup>, R<sup>32</sup>, R<sup>33</sup>, R<sup>34</sup>, R<sup>37</sup> and R<sup>38</sup> (same or different) being selected from the group consisting of hydrogen, halogen, an alkyl group or an aryl group, and each of R<sup>35</sup> and R<sup>36</sup> (same or different) represents hydrogen, an alkyl group, an aryl group

or together represent the necessary atoms to close a cycloaliphatic ring.

15. An electrophotographic recording material according to claim 1, wherein the polymeric binder consists of a combination of an aromatic polycarbonate and a copolyester of terephthalic acid and isophthalic acid with ethylene glycol and neopentyl glycol, the molar ratio of tere- to isophthalic acid being 3/2.

16. An electrophotographic recording material ac-

cording to claim 1, wherein the n-type pigment substance is 4,10-dibromoanthanthrone.

17. An electrophotographic recording material according to claim 1, wherein the p-type charge transport substance is 1,2-bis(1,2-dihydro-2,2,4-trimethyl-quinolin-1-yl)ethane.

\* \* \* \* \*

10

15

20

25

30

35

40

45

50

55

60

65